



US005460916A

**United States Patent**

[19]

**Iwasaki**[11] **Patent Number:** **5,460,916**[45] **Date of Patent:** **Oct. 24, 1995****[54] SILVER HALIDE PHOTOGRAPHIC MATERIAL AND METHOD OF FORMING RADIATION IMAGE USING SAID MATERIAL****[75] Inventor:** **Nobuyuki Iwasaki**, Kanagawa, Japan**[73] Assignee:** **Fuji Photo Film Co., Ltd.**, Kanagawa, Japan**[21] Appl. No.:** **248,245****[22] Filed:** **May 24, 1994****[30] Foreign Application Priority Data**

May 24, 1993 [JP] Japan ..... 5-121675

**[51] Int. Cl.<sup>6</sup>** ..... **G03C 5/16****[52] U.S. Cl.** ..... **430/139; 430/502; 430/567;**  
**430/967; 430/435****[58] Field of Search** ..... **430/502, 139,**  
**430/567, 967, 435****[56] References Cited****U.S. PATENT DOCUMENTS**

|           |         |                  |       |         |
|-----------|---------|------------------|-------|---------|
| 4,425,426 | 1/1984  | Abbott et al.    | ..... | 430/502 |
| 4,439,520 | 3/1984  | Kofron et al.    | ..... | 430/502 |
| 4,639,417 | 1/1987  | Honda et al.     | ..... | 430/567 |
| 4,689,292 | 8/1987  | Metoki et al.    | ..... | 430/567 |
| 4,803,150 | 2/1989  | Dickerson et al. | ..... | 430/502 |
| 5,108,881 | 4/1992  | Dickerson et al. | ..... | 430/502 |
| 5,252,442 | 10/1993 | Dickerson et al. | ..... | 430/502 |
| 5,268,251 | 12/1993 | Sakuma           | ..... | 430/139 |

**Primary Examiner**—Thomas R. Neville**Attorney, Agent, or Firm**—Sughrue, Mion, Zinn, Macpeak & Seas**[57] ABSTRACT**

Disclosed is a silver halide photographic material for X-ray photography which has at least one light-sensitive silver

halide emulsion layer on each side of a transparent support and constitutes a radiation image-forming system in combination with two radiation-intensifying screens respectively arranged on the front and the back sides of the photographic material. The photographic material is characterized by having a crossover rate of at most 15% with respect to the light emitted from said intensifying screens, and by producing an image having a characteristic curve such that when drawn using crossed coordinates equal to each other in unit length, with diffusion density as ordinate (Y-axis) and common logarithm of exposure amount as abscissa (X-axis), the characteristic curve provides a point gamma value ranging from 2.7 to 4.2 at every point within the optical density (diffusion density) range of 1.6 to 2.0 and a point gamma value of at least 0.25 at the density point corresponding to  $\frac{1}{10}$  of the exposure amount (-1.0 on logarithmic scale) required for providing the optical density of 1.8 when sandwiched between two intensifying screens having substantially the same sensitivity, subjected to stepwise exposure and then developed with Developer (I) having the following composition at a developer temperature of 35° C. for a development time of 25 seconds:

**Composition of Developer (I)**

|                         |        |
|-------------------------|--------|
| Potassium hydroxide     | 21 g   |
| Potassium sulfite       | 63 g   |
| Boric acid              | 10 g   |
| Hydroquinone            | 25 g   |
| Triethylene glycol      | 20 g   |
| 5-Nitroindazole         | 0.2 g  |
| Glacial acetic acid     | 10 g   |
| 1-Phenyl-3-pyrazolidone | 1.2 g  |
| 5-Methylbenzotriazole   | 0.05 g |
| Glutaraldehyde          | 5 g    |
| Potassium bromide       | 4 g    |
| Water to make           | 1 l    |
| pH adjusted to          | 10.02  |

**14 Claims, 1 Drawing Sheet**



**SILVER HALIDE PHOTOGRAPHIC  
MATERIAL AND METHOD OF FORMING  
RADIATION IMAGE USING SAID  
MATERIAL**

**FIELD OF THE INVENTION**

The present invention relates to a novel silver halide photographic material and to a method of forming an X-ray image. In particular, the present invention is concerned with a silver halide photographic material which can provide an image of excellent quality in the field of X-ray photography for the thoracic diagnosis and with a method for forming said image.

**BACKGROUND OF THE INVENTION**

In medical radiography, the image of affected tissue of a patient is formed by recording the pattern of X rays transmitted by the tissue in a photosensitive material which comprises a transparent support having thereon at least one light-sensitive silver halide emulsion layer (i.e., a silver halide photographic material). A transmission pattern of X rays can be recorded by using a silver halide photographic material alone. However, it is undesirable for the human body to be exposed to X rays in quantity, so that a combination of a silver halide photographic material with a radiation intensifying screen is generally used in practicing X-ray photography. The radiation intensifying screen comprises a support having a phosphor layer provided thereon, and the phosphor layer functions so as to convert the X rays absorbed thereby to visible rays to which a silver halide photographic material has high sensitivity. Therefore, the intensifying screen can markedly improve the sensitivity of an X-ray photograph taking system.

For the purpose of further heightening the sensitivity of an X-ray photograph taking system, there was developed the method of using a both-sided emulsion film, or a silver halide photographic material having silver halide light-sensitive emulsion layers on front and back sides of a support respectively, and practicing X-ray photography in a condition such that the film is inserted between two radiation intensifying screens (which may be simply called "intensifying screen"). In ordinary X-ray photography, the above-described photograph taking method is adopted at present. The development of this method originated in that sufficient X-ray absorption was not achieved by the use of only one intensifying screen. More specifically, even if the amount of a phosphor contained in one intensifying screen is increased, the converted visible rays are scattered and reflected inside the phosphor layer since the increased content of the phosphor results in thickening the phosphor layer. Accordingly, the visible rays emitted from the intensifying screen strike divergently on the surface of the photosensitive material disposed in contact with the intensifying screen. In addition, the visible rays generating in the depth of the phosphor layer are hard to get out of the phosphor layer. Thus, the amount of effective visible rays emitted from the intensifying screen cannot be increased even if the thickness of the phosphor layer is increased excessively. On the other hand, the X-ray photograph taking method using two intensifying screens which each contain a phosphor layer having a moderate thickness has an advantage in that the X-ray absorption as a whole can be increased and effectively converted visible rays can be taken out of the intensifying screens.

The research for finding out an X-ray photograph taking system excellent in balance between image quality and

photographic speed has so far been carried out continuously. For instance, there has been prevailingly used the combination of a blue light-emitting intensifying screen having a layer containing calcium tungstate as a phosphor with a spectrally unsensitized silver halide photographic material (e.g., the combination of Hi-Screen Standard and RX, both being the products of Fuji Photo Film Co., Ltd.). In recent years, however, the combination of a green light-emitting intensifying screen having a layer containing the terbium-activated oxysulfide of a rare earth element as a phosphor with an orthochromatically sensitized silver halide photographic material (e.g., the combination of Grenex 4 with RXO, both being the products of Fuji Photo Film Co., Ltd.) has come to be used, and has effected improvements in both sensitivity and image quality.

However, a silver halide photographic material provided with photographic emulsion layers on both sides has a problem of tending to suffer deterioration in image quality due to crossover rays. The term "crossover rays" used herein refers to the visible rays which are emitted from each of the intensifying screens arranged on both sides of a photosensitive material, are transmitted by the support (usually having a thickness of 170-180  $\mu\text{m}$  or so) of the photosensitive material and further reach the light-sensitive layer disposed on the opposite side, thereby causing deterioration in image qualities (especially sharpness).

For the purpose of reducing the above-described crossover rays, various arts have so far been developed. For instance, U.S. Pat. Nos. 4,425,425 and 4,425,426 disclose the arts of using spectrally sensitized tabular-grain emulsions having high aspect ratios as light-sensitive silver halide photographic emulsions. According to those inventions, it is possible to reduce the crossover rays to 15-22%. Moreover, U.S. Pat. No. 4,803,150 discloses the art of disposing a layer of a microcrystalline dye capable of being decolored by development-processing between the support and the light-sensitive layer of a silver halide photographic material. Such an invention enables the crossover rays to be reduced to below 10%.

The gradation of photographs (characteristic curve's shape) is very important at the time of making medical diagnoses using photographic images. Recently, it has been diagnosticians' study to properly use photographic materials according to the portion to be diagnosed in human body. Following this trend, photographic film makers provide photosensitive materials various in their characteristic curves. The photosensitive materials on the market today are roughly classified into high contrast photosensitive materials for blood vessel contrasting photography, standard contrast photosensitive material for amateur use, wide latitude photosensitive materials for photographing abdomen and stomach, extremely wide latitude photosensitive materials for photographing thorax, and so on.

Further, various photosensitive materials differing in characteristic curve are disclosed in JP-A-59-214027 (the term "JP-A" as used herein means an "unexamined published Japanese patent application"), JP-A-60-41035, JP-A-60-159741, JP-A-61-116346, JP-A-62-42146, and JP-A-62-42147.

On the other hand, there have been made attempts to find out X-ray photograph taking systems excellent in balance between image quality and photographic speed by combining a silver halide photographic material having photographic emulsions on both sides thereof with radiation intensifying screens under specified conditions. For instance, JP-A-02-266344, JP-A-02-297544 and U.S. Pat.

No. 4,803,150 disclose the X-ray photographing systems designed so that the combination of an intensifying screen arranged on the X-ray irradiation side (front intensifying screen) with a light-sensitive layer (front sensitive layer) may be different in spectral characteristic (sensitivity) from the combination of an intensifying screen arranged on the opposite side (back intensifying screen) with a light-sensitive layer (back sensitive layer) and, what is more, the front combination and the back combination may have different contrasts. Further, experimental results of the combinations of the products of 3M Co., Ltd. concerning silver halide photographic materials and radiation intensifying screens are reported in *Photographic Science and Engineering*, Vol. 26, No. 1, p. 40 (1982). More specifically, the report states that the combination of Trimax 12 (trade name, a commercial intensifying screen of 3M Co.) with XUD (trade name, a commercial silver halide photographic material of 3M Co.) is almost equal in sensitivity and sharpness (MTF) to the combination of Trimax 4 (trade name, a commercial intensifying screen of 3M Co.) with XD (trade name, a commercial silver halide photographic material), but the former combination is higher in NEQ (ratio of noise to output signal) than the latter. Further, the report teaches that the above-described results can be inferred from the fact that XUD shows higher sharpness than XD, while Trimax 12 shows higher X-ray absorption than Trimax 4.

If attention is devoted only to the quality of X-ray images, it goes without saying that high quality images can be obtained by the combined use of a low-sensitivity silver halide photographic material and low-sensitivity radiation intensifying screens. In using a low-sensitivity combination as described above, however, it becomes indispensable to increase an amount of X rays to which human body is exposed (exposure amount). Consequently, such a combination is undesirable for practical use. In the case of a mass examination in particular, wherein most of the subjects are healthy persons, it is impossible to use that combination in practice because it is necessary to strictly avoid an increase in exposure amount.

As described above, there have so far been conducted researches for finding out various types of X-ray photograph taking systems which can provide excellent balance between image quality and photographic speed. However, hitherto developed X-ray image forming methods cannot be yet said to be embodied in X-ray photograph taking systems endowed with image quality and sensitivity high enough for the purpose of thoracic diagnoses using X-ray images. As for the X-ray image of thorax, for instance, it is very important from the diagnostic point of view that the shadow of very thin blood vessels in the lung field can be observed up to their terminal parts. However, conventional X-ray photograph taking systems cannot satisfy such a requirement.

Moreover, another difficulty comes up in photographing the thorax of human body. More specifically, the thorax is photographed using X rays in order to diagnose mainly lungs as a whole, and the X-ray photograph thereof has to depict coextensively a thoracic part by which X rays are transmitted in a relatively large quantity, including middle and upper areas of lungs, and a thoracic part by which X rays are transmitted in an extremely small quantity, including the central shadowy, heart and subphrenic areas. The difference in quantity of the transmitted X-rays, as described in *SPIE*, vol. 1651 entitled "Medical Imaging VI: Instrumentation" (1992), becomes greater the fatter physique the photographed person has, and it ranges specifically from 0.9 to 1.1 in terms of the logarithm of the difference in exposure amount. Accordingly, it is necessary for a screen/film system

to widen its dynamic range (latitude). However, widening the latitude is contradictory to high contrast requirements.

Therefore, only one sheet of photograph taken by a hitherto known method for photographing a thorax with X rays cannot provide wholly satisfactory image information to diagnosticians. That is, the image obtained using a thorax photograph taking system of wide-latitude type, though contrasty in the areas by which X rays were transmitted in a small quantity, such as in the central shadowy and subphrenic areas, is hard to view and to serve diagnosis because the overall impression is one of roughness with the grain coarseness standing out, and the shadow of blood vessels in the lung field is short of contrast and sharpness.

On the other hand, when a photosensitive material of standard gradation is used, the shadow of blood vessels in the lung field has satisfactory contrast, but the image obtained is hard to serve diagnosis because it gives the impression of being one of roughness with the grain coarseness standing out. In addition, the image obtained wants depiction of the central shadowy area and the like, so it is quite inferior in quality. For the purpose of making an improvement in depiction of the central shadowy area and the like, there can be adopted a method of photographing with X rays emitted under a high pressure condition. However, such a method can only provide images having on the whole low contrast and lacking sharpness through the influence of scattered rays. Although an improvement in depiction of the central shadowy area and the like can also be brought about using another method of increasing the exposure amount, the image density in the lung field becomes so high that diagnosis cannot be easily made by the observation with a generally used Schaukasten.

#### SUMMARY OF THE INVENTION

A primary object of the present invention is to provide a silver halide photographic material which constitutes a novel system for taking X-ray photographs excellent in balance between image quality and photographic speed.

Another object of the present invention is to provide a silver halide photographic material which constitutes a novel system for providing X-ray photographs having excellent qualities, especially for taking a photograph of the thorax.

A further object of the present invention is to provide a X-ray photograph taking method in which the combination of a novel silver halide photographic material and a radiation screen provides an image used to greater advantage.

As a result of intensive studies, it has been found out that the above-described objects can be attained by using a silver halide photographic material for X-ray photography which has at least one light-sensitive silver halide emulsion layer on each side of a transparent support and constitutes a radiation image-forming system comprising two radiation-intensifying screens respectively arranged on the front and the back sides of the photographic material; said photographic material having a crossover rate of at most 15% with respect to the light emitted from said intensifying screens and, when sandwiched between two intensifying screens having substantially the same sensitivity, subjected to step-wise exposure and then developed with Developer (I) having the following composition at a developer temperature of 35° C. for a development time of 25 seconds, said photographic material producing an image having a characteristic curve such that when drawn using crossed coordinates equal to each other in unit length, with diffusion density as ordinate (Y-axis) and common logarithm of exposure amount as

abscissa (X-axis), the characteristic curve provides a point gamma value ranging from 2.7 to 4.2 at every point within the optical density (diffusion density) range of 1.6 to 2.0 and a point gamma value of at least 0.25 at the density point corresponding to  $1/10$  of the exposure amount ( $-1.0$  on logarithmic scale) required for providing the optical density of 1.8:

| Composition of Developer (I) |        |
|------------------------------|--------|
| Potassium hydroxide          | 21 g   |
| Potassium sulfite            | 63 g   |
| Boric acid                   | 10 g   |
| Hydroquinone                 | 25 g   |
| Triethylene glycol           | 20 g   |
| 5-Nitroindazole              | 0.2 g  |
| Glacial acetic acid          | 10 g   |
| 1-Phenyl-3-pyrazolidone      | 1.2 g  |
| 5-Methylbenzotriazole        | 0.05 g |
| Glutaraldehyde               | 5 g    |
| Potassium bromide            | 4 g    |
| Water to make                | 1 l    |
| pH adjusted to               | 10.02  |

#### BRIEF DESCRIPTION OF THE DRAWING

FIGURE illustrates a characteristic curve of a photographic light-sensitive material prepared in accordance with an embodiment of the present invention. Therein, a curve connecting point gamma values at individual points on the characteristic curve (gamma curve) is also shown.

In FIGURE, the exposure amount ( $\log E$ ) is plotted as abscissa and the optical density or the gamma value as ordinate, and numeral 1 indicates the characteristic curve and numeral 2 the gamma curve.

#### DETAILED DESCRIPTION OF THE INVENTION

The term "crossover" used herein means the rays which are some portion of the rays incident upon one emulsion layer of a photographic material having light-sensitive emulsions coated on both sides of a transparent support, and correspond to those transmitted by said emulsion layer and the support to sensitize the other emulsion layer on the opposite side. The crossover rate (%) can be determined by the method disclosed by U.S. Pat. No. 4,425,425 to Abbott et al. Specifically, black paper, a photosensitive material having substantially the same light-sensitive layers on both sides and a intensifying screen are superposed upon one another, in that order starting from the X-ray source, packed in a cassette for X-ray photography, and exposed stepwise to X rays. After development, the photosensitive material is divided into two pieces, only the light-sensitive layer which has been in contact with the intensifying screen is left in one piece and the image formed therein is examined for characteristic curve. In the other piece, on the other hand, only the light-sensitive layer on the opposite side is left and the image formed therein is examined for characteristic curve. Thus, the crossover rate (%) is defined as follows, with a difference in sensitivity between these two characteristic curves in the density region corresponding to the nearly linear portion being taken as  ${}^A \log E$ :

$$\text{Crossover rate (\%)} = 100 / (\text{anti log} ({}^A \log E) + 1)$$

The lower the crossover rate of a photographic material is, the sharper image the material can form. Various methods of

reducing crossover are known. The most desirable method consists in fixation of a dye of the type which can be decolored by development between a support and a light-sensitive material. The microcrystalline dyes taught by U.S. Pat. No. 4,803,150 have great advantage in reducing crossover because they can be fixed to a satisfactory extent, decolored completely, and contained in quantities.

According to such a method, not only desensitization due to unsatisfactory fixation does not occur, but also the dyes can be decolored even by 90-second development and the crossover rate can be reduced to at most 15%.

As for the dye layer provided for reducing crossover, a layer having the highest possible dye density is favored. Further, it is desirable that the coverage of gelatin used as binder in the dye layer be reduced and the thickness of the dye layer be set at 0.5  $\mu\text{m}$  or less. However, when the dye layer is rendered too thin, it tends to cause a poor adhesion trouble. Therefore, the most suitable thickness of the dye layer ranges from 0.05 to 0.3  $\mu\text{m}$ .

Photographic materials having their characteristic curves within the scope of the present invention can provide images enabling easy diagnosis of thorax. More specifically, the point gamma values corresponding to the density range of 1.6 to 2.0 are within the range of 2.7 to 4.2, that is, rather hard images are obtained and a sharp contrast is made between light and shadow areas in the lung field. Thus, the image of blood vessels and the shadow of a tumor can be clearly observed in the thoracic image obtained. Moreover, the images obtained is free from blur caused by crossover, so that even the details thereof can be observed distinctly. In addition, a blank in the image is not made even in low density areas, such as the central shadowy part and so on, since the point gamma values in low-exposure areas are also relatively high.

The term "point gamma" used in the present invention is defined as follows: At a given point on a characteristic curve, which is drawn using crossed coordinates equal to each other in unit length, with diffusion density as ordinate (Y-axis) and common logarithm of exposure amount as abscissa (X-axis), the tangent is drawn and the slope thereof is defined as point gamma. That is, when the angle the tangent forms with the X-axis is  $\theta$ , the point gamma is represented by  $\tan\theta$ .

The characteristic curve according to the present invention and the differential curve thereof are shown in FIGURE.

The standard condition for photographic processing using Developer (I) is described below in detail.

Development time: 25 seconds (21 seconds inside the developer+4 seconds outside the developer)

Fixation time: 20 seconds (16 seconds inside the fixer having the following composition+4 seconds outside the fixer)

Washing time: 12 seconds

Squeeze and Drying: 26 seconds

Developing Machine: A commercial model of roller conveyable type automatic developing machine (e.g., Auto Processor Model FPM-5000, made by Fuji Photo Film Co., Ltd.) equipped with a developing tank having a volume of 22 l and a developer temperature of 35° C. and a fixing tank having a volume of 15.5 l and a fixer temperature of 25° C. As another commercial model of automatic developing machine of the same type as described above, Auto Processor Model M-6AW, made by Eastman Kodak Co., Ltd., is instanced.

## Composition of Fixer (Fixer F):

|                                                  |        |
|--------------------------------------------------|--------|
| Ammonium thiosulfate (70% weight/volume)         | 200 ml |
| Sodium sulfite                                   | 20 g   |
| Boric acid                                       | 8 g    |
| Disodium ethylenediaminetetraacetate (dihydrate) | 0.1 g  |
| Aluminum sulfate                                 | 15 g   |
| Sulfuric acid                                    | 2 g    |
| Glacial acetic acid                              | 22 g   |
| Water to make                                    | 1 l    |

Fixer F is adjusted to pH 4.5 using sodium hydroxide or glacial acetic acid, if needed.

A photosensitive material having its characteristic curve within the scope of the present invention can be obtained in various ways. An appropriate way to obtain the material is illustrated below:

Firstly, two kinds of emulsions differing in sensitivity are chosen. As for the sensitivity difference between the emulsions chosen, it is desirable that the ratio of the sensitivity of one emulsion to that of the other be in the range of 1:0.5 to 1:0.15. These two emulsions may be coated together in a single layer, or they may be coated separately in a double layer. In the most desirable embodiment, the high-speed emulsion constitutes the upper layer and the low-speed emulsion the lower layer. The ratio of the coverage of the high-speed emulsion to that of the low-speed emulsion ranges from 0.5:1 to 0.05:1, preferably from 0.3:1 to 0.1:1, based on silver. As for the low-speed emulsion, it is desirable that the grain size distribution thereof be monodisperse. When the variation coefficient (%) is defined as 100 times the quotient of the standard deviation of grain sizes divided by an average grain size, emulsions having a variation coefficient of at most 20% with respect to the grain size distribution are preferred as the low-speed emulsion.

A representative of the silver halide photographic materials in accordance with the present invention has a construction such that a subbing layer, a dye layer for reduction of crossover, at least one light-sensitive silver halide emulsion layer and a protective layer are formed in that order on each of the front and back sides of a blue-colored transparent support. Preferably, every couple of corresponding layers formed on both sides are substantially the same as each other.

The support is made from a transparent material such as polyethylene terephthalate, and colored with a blue dye. As for the blue dye, various kinds of dyes including anthraquinone dyes known as the dyes for coloring X-ray photographic films can be used. The thickness of the support can be properly chosen from the range of 160 to 200  $\mu\text{m}$ .

On the support, in analogy with conventional X-ray photographic films, a subbing layer comprising a water-soluble high molecular substance such as gelatin is provided.

On the subbing layer, a dye layer for reduction of crossover is provided. The dye layer is generally formed as a dye-containing colloid layer, and it is desirable that the dye layer be decolored by the development-processing defined above. Further, it is desirable that the dye be fixed to the bottom of the dye layer so as not to diffuse into the upper layers including a light-sensitive silver halide emulsion layer and a protective layer.

On the dye layer, a light-sensitive silver halide emulsion layer is formed. Light-sensitive silver halide emulsions used in the photosensitive material of the present invention can be prepared in known manners.

In addition, it is required of the photosensitive material to

have sensitivity to an intensifying screen used together therewith. Since ordinary silver halide emulsions have their sensitivities to light of wavelengths ranging from those of blue rays to those of ultraviolet rays, the foregoing point can be left out of consideration in so far as the wavelengths of rays emitted from the intensifying screen are within the wavelength region of blue to ultraviolet rays (e.g., as in the case of using an intensifying screen containing a phosphor a calcium tungstate phosphor). However, when an intensifying screen using, e.g., a terbium-activated gadolinium oxysulfide phosphor emitting rays having their main wavelength at 545 nm is employed, spectral sensitization in the green region is required of the silver halide grains contained in the photosensitive material.

Silver halide emulsions which can be preferably used in the silver halide photographic material of the present invention are emulsions containing tabular silver halide grains. This is because the emulsions containing tabular silver halide grains have advantages in that they are well balanced between sensitivity and granularity, have excellent spectral sensitization characteristics and great ability to reduce crossover, and so on.

In recent years, various improvements have been introduced in the methods of preparing an emulsion containing tabular silver halide grains. Those arts of improving the preparation methods can be also adopted in preparing tabular-form silver halide emulsion grains used for producing the silver halide photographic material of the present invention. Specific examples of such arts include the art of improving the pressure characteristics of tabular silver halide grains by combining reduction sensitization with the addition of a mercapto compound or a certain dye, the art of sensitizing tabular silver halide grains with a selenium compound, the art of reducing the pressure mark generating upon roller conveyance by decreasing an iodide content in surface part of the individual grains, and the art of improving the balance between the reduction in pressure mark upon roller conveyance and drying characteristics by adjusting the silver/gelatin ratio in each layer to a most appropriate value when the photographic material has a double-layer emulsion structure. The above-cited arts are disclosed in JP-A-4-344635, JP-A-5- 45754, JP-A-3-288145, JP-A-4-163447, JP-A-4-107442 and JP-A- 4-311949.

As described above, it is desirable that the dye layer which is a constituent layer of the present silver halide photographic material be decolored under the aforementioned development condition. In order to carry out this purpose, it is advantageous to decrease the amount of a binder used in the light-sensitive layer disposed on the dye layer. Specifically, it is desirable to control the binder content in the light-sensitive layer 5 g/m<sup>2</sup> or less, preferably 3 g/m<sup>2</sup> or less. On the other hand, the content of silver in the light-sensitive layer is preferably adjusted to at most 3 g/m<sup>2</sup>, particularly at most 2 g/m<sup>2</sup>.

On the laminate thus formed on each side of a support, including a subbing layer and a light-sensitive layer, a protective layer comprising a water-soluble high molecular substance, such as gelatin, is provided in a conventional manner, thereby obtaining the silver halide photographic material of the present invention.

The silver halide photographic material according to the present invention does not have any particular limitation as to the emulsion sensitization method, additives and ingredients used for the preparation thereof, the photographic processing method to which it is subjected. For instance, various arts as described in JP-A-02-68539, JP-A-02-103037 and JP-A-02-115837 can be used, which are

summarized below with pages on which they are specifically described.

| Item                                     | Reference                                                                                                                                                                                              |
|------------------------------------------|--------------------------------------------------------------------------------------------------------------------------------------------------------------------------------------------------------|
| 1. Chemical sensitization                | JP-A-02-68539, page 10, from right upper column, line 13, to left lower column, line 16.                                                                                                               |
| 2. Antifoggant, Stabilizer               | JP-A-02-68539, from page 10, left lower column, line 17, to page 11, left upper column, line 7, and from page 3, left lower column, line 2, to page 4, left lower column.                              |
| 3. Spectral sensitizing dye              | JP-A-02-68539, from page 4, right lower column, line 4, to page 8, right lower column.                                                                                                                 |
| 4. Surfactant, Antistatic agent          | JP-A-02-68539, from page 11, left upper column, line 14, to page 12, left upper column, line 9.                                                                                                        |
| 5. Matting agent, Lubricant, Plasticizer | JP-A-02-68539, page 12, from left upper column, line 10, to right upper column, line 10, and page 14, from left lower column, line 10, to right lower column, line 1.                                  |
| 6. Hydrophilic colloid                   | JP-A-02-68539, page 12, from right upper column, line 11, to left lower column, line 16.                                                                                                               |
| 7. Hardener                              | JP-A-02-68539, from page 12, left lower column, line 17, to page 13, right upper column, line 6.                                                                                                       |
| 8. Support                               | JP-A-02-68539, page 13, right upper column, from line 7 to line 20.                                                                                                                                    |
| 9. Dye, Mordant                          | JP-A-02-68539, from page 13, left lower column, line 1, to page 14, left lower column, line 9.                                                                                                         |
| 10. Photographic processing              | JP-A-02-103037, from page 16, right upper column, line 7, to page 19, left lower column, line 15, and JP-A-02-115837, from page 3, right lower column, line 5, to page 6, right upper column, line 10. |

Further, preferred embodiments of the present invention are described in detail.

It has proved that good image quality and satisfactory photographic speed can be obtained when the silver halide photographic material having a novel characteristic curve defined by the present invention and a reduced crossover rate possesses its sensitivity in a specified range and is used for image formation in combination with intensifying screens of the kind which have high sensitivity and relatively good contrast transfer function (CTF), namely the CTF value of at least 0.79 at a spacial frequency of 1 line/mm and the CTF value of at least 0.36 at a spacial frequency of 3 lines/mm.

That is, although a photographic material and intensifying screens may be arbitrarily combined, more improved balance can be acquired between the image quality and the photographic speed when the combination satisfying the above-described sensitivity and contrast requirements is adopted. On the condition that the photographic speed of the combined system is constant, when high-sensitivity intensifying screens which can absorb X rays in considerable quantities are used in combination with a photosensitive material of low sensitivity, the image obtained is very excellent in granularity but quite inferior in sharpness. Even when the photosensitive material used in the above case has high sharpness, the image obtained does not have satisfac-

tory sharpness and cannot be a desirable X-ray image from the diagnostic point of view. Conversely, when low-sensitivity intensifying screens having poor X-ray absorption are used in combination with a photosensitive material of standard or high sensitivity, an X-ray image of high sharpness can be obtained, but the image suffers from deterioration of granularity. In this case also, therefore, the X-ray image obtained is undesirable from the viewpoint of diagnosis. The best combination is obtained by combining intensifying screens of the kind which have relatively high sensitivity such that they have X-ray absorption of at least 25% when irradiated with the X rays of 80 KVp and have CTF values of at least 0.79 at a spacial frequency of 1 line/mm and at least 0.36 at a spacial frequency of 3 lines/mm with a photosensitive material having a sensitivity reduced to such an extent that the high sensitivity characteristics of the intensifying screens can be canceled out by the sensitivity reduction of the photosensitive material.

According to our study, it proved that most suitable sensitivity distribution in the combined system of a silver halide photographic material and radiation intensifying screens depends on the photographic speed level of the combined system, the size of a subject for diagnosis and so on. As a result of further study, however, we have found that an X-ray image of high quality can be obtained with sufficiently high photographic speed when a photosensitive material having moderate sensitivity is used in combination with intensifying screens in which the content of a phosphor is increased to such an extent that it is possible to keep allowable level of sharpness in order to increase the amount of X rays absorbed thereby, and which are designed so as to exhibit high contrast transfer function (CTF) values.

In the meantime, the preferred level of sharpness depends on the size of a subject for diagnosis. In making clinical evaluation of thorax, the contrast transfer function values at spacial frequencies ranging from 0.5 line/mm to 3 lines/mm are important when the evaluation is expressed in terms of contrast transfer function (CTF) as a physical quantity. More specifically, it is required that the value of contrast transfer function at the spacial frequency of 1 line/mm is at least 0.65 and that at the spacial frequency of 2 lines/mm is at least 0.22. In addition, there are restrictions as to the photographic speed of the combined system. This is because if the system having high photographic speed as a whole is chosen, image quality high enough to diagnose thorax or the like cannot be obtained even if the system is composed so as to acquire the most desirable balance. Conversely, the system of low photographic speed is undesirable because it creates an X-ray exposure problem.

The expression "specific sensitivity range which favors the silver halide photographic material" refers to the sensitivity range requiring the exposure amount ranging from 0.010 lux-sec to 0.035 lux-sec, preferably 0.012 to 0.030 lux-sec to provide the density of minimum density plus 0.5 for the light-sensitive layer disposed on the exposure side when the photographic material is exposed to monochromatic light having the same wavelength as that of the main emission peak of the radiation intensifying screens and a half width of  $20\pm 5$  nm, developed with Developer (I) described hereinbefore under a condition that a developer temperature is regulated at 35° C. and a development time is set at 25 seconds, and examined for the image density after the light-sensitive layer disposed on the side opposite to the exposure side is removed therefrom.

The sensitivities set within the above-described range are lower than the sensitivities of commercially available X-ray films, such as Roentgen Film Super HRS, products of Fuji

Photo Film Co., Ltd.

In measuring the sensitivity of the silver halide photographic material, it is necessary to use the exposure light source whose wavelength coincides with or almost coincides with the wavelength of the main emission peak of the radiation intensifying screens used in combination with the photographic material. For instance, when the phosphor of the radiation intensifying screen is terbium-activated gadolinium oxysulfide, the wavelength of the main emission peak thereof is 545 nm. Accordingly, a light source used in measuring the sensitivity of the silver halide photographic material is one which can emit light of wavelengths centering at 545 nm.

In order to obtain monochromatic light, a method of using a filter system constituted of a light source and interference filter(s) can be adopted. According to this method, though the intensity and the half width of monochromatic light depend on what kinds of interference filters are combined with a light source, monochromatic light having intensity high enough to provide the required amount of exposure and a half width of  $20 \pm 5$  nm can be generally obtained with ease. Additionally, the silver halide photographic material shows a continuous spectrum with respect to its spectral sensitivities, irrespective of its being spectrally sensitized or not. Therefore, it can be said that the sensitivities are substantially constant in the wavelength range of  $20 \pm 5$  nm.

As an example of an exposure light source, the system constituted of a tungsten light source (color temperature: 2856° K.) and a transmitting filter having a transmission peak at the wavelength of 545 nm and a half width of 20 nm can be used when the phosphor in the radiation intensifying screen used in combination with the photographic material is terbium-activated gadolinium oxysulfide.

Then, radiation intensifying screens which can be used to advantage in the present invention are illustrated in detail.

The radiation intensifying screens used in the combined system of the present invention can be easily obtained by designing so as to acquire the sensitivity defined by the present invention and carrying out the preparation thereof according to conventional arts of preparing radiation intensifying screens. Specific examples of intensifying screens are described in *Research Disclosure*, Item 18431, Section IX.

The radiation intensifying screen is basically constituted of a support and a phosphor layer formed on one side thereof. The phosphor layer is a layer containing a phosphor dispersed in a binder. In addition, a transparent protective layer is generally provided on the surface of the phosphor layer (the side opposite to the support) to protect the phosphor layer from chemical change in quality and physical impact.

Phosphors which can be preferably used for the radiation intensifying screens in the present invention are represented by the following general formula:



wherein M represents at least one metal selected from a group consisting of yttrium, lanthanum, gadolinium and lutetium; M' represents at least one rare earth element, preferably dysprosium, erbium, europium, holmium, neodymium, praseodymium, samarium, cerium, terbium, thulium or ytterbium; X represents an intermediate chalcogen (S, Se or Te) or a halogen; n is a numerical value ranging from 0.0002 to 0.2; and w is 1 when X is a halogen, while it is 2 when X is a chalcogen.

Specific examples of a radiation intensifying phosphor which can be preferably used in the radiation intensifying

screens of the present invention include terbium-activated rare earth metal oxysulfide type phosphors [e.g.,  $Y_2O_3S:Tb$ ,  $Gd_2O_3S:Tb$ ,  $La_2O_3S:Tb$ ,  $(Y,Gd)_2O_3S:Tb$ ,  $(Y,Gd)_2O_3S:Tb$ ,  $Tm$ ], terbium-activated rare earth element oxyhalogenide type phosphors [e.g.,  $LaOBr:Tb$ ,  $LaOBr:Tb,Tm$ ,  $LaOCl:Tb$ ,  $LaOCl:Tb,Tm$ ,  $GdOBr:Tb$ ,  $GdOCl:Tb$ ] and thulium-activated rare earth element oxyhalogenide type phosphors [e.g.,  $LaOBr:Tm$ ,  $LaOCl:Tm$ ].

Of these phosphors, terbium-activated gadolinium oxysulfide type phosphor is particularly preferred as a phosphor for the radiation intensifying screens used in the present invention. The phosphor of the foregoing type is described in detail in U.S. Pat. No. 3,725,704.

The phosphor layer is generally provided on a support under ordinary pressure using a coating method as described below. Specifically, the phosphor layer is formed in a manner such that granulated phosphor and a binder are mixed and dispersed in an appropriate solvent to prepare a dispersion, the dispersion prepared is directly applied to a support for radiation intensifying screen using a coating means, such as a doctor blade, a roll coater, a knife coater, etc., under ordinary pressure, and then the solvent is removed from the coating. In another manner, the foregoing dispersion is coated in advance on a temporary support, such as a glass plate, under ordinary pressure, the solvent is removed from the coating to form a thin film of phosphor-containing resin, and then the thin film is peeled apart from the temporary support and bonded to the support for a radiation intensifying screen.

In preparing the radiation intensifying screens used in the present invention, though a conventional manner as described above can be adopted, it is preferable to use a thermoplastic elastomer as a binder and to undergo a compressive stressing treatment in order to heighten the packing rate of a phosphor (that is, to lessen the voids in the phosphor layer).

The sensitivity of the radiation intensifying screen depends basically upon the total amount of emission from the phosphor contained in the panel, and the total amount of emission depends upon not only the emission luminance of the phosphor itself but also the phosphor content in the phosphor layer. A high phosphor content means that a large amount of radiation, such as X rays, can be absorbed by the phosphor. Therefore, the higher the phosphor content, the higher sensitivity the intensifying screen can have, and at the same time it can contribute to improvements in image quality (especially in graininess). If the phosphor content in a phosphor layer is set at some definite value, on the other hand, relatively higher sharpness can be achieved the more densely the phosphor grains are packed. This is because denser packing of the phosphor grains can make the phosphor layer thinner, thereby reducing the divergence of emitted rays due to scattering phenomenon.

A suitable process of preparing the above-described type of radiation intensifying screens comprises:

- (a) a step of forming a phosphor sheet containing a binder and a phosphor, and
- (b) a step of putting the foregoing phosphor sheet on a support and binding the sheet to the support as the sheet is compressively stressed at a temperature higher than the softening point or melting point of the binder.

Firstly the step (a) is illustrated.

A phosphor sheet which serves as the phosphor layer of a radiation intensifying screen can be prepared by coating a composition prepared by dispersing phosphor grains homogeneously into a binder solution on a temporary support for phosphor sheet formation, drying the composition coated,

and then peeling it off the temporary support.

More specifically, a binder and phosphor grains are added to an appropriate organic solvent, and mixed with stirring to disperse the phosphor grains homogeneously into a binder solution. Thus, the coating composition is prepared.

As the binder, a thermoplastic elastomer having its softening or melting point in the temperature range of 30° C. to 150° C. can be used alone, or as a mixture with another binder polymer. Since thermoplastic elastomers have elasticity at ordinary temperature and come to have flowability by heating, they can protect the phosphor grains from being broken by pressure applied thereto upon compressive stressing. Specific examples of a thermoplastic elastomer include polystyrene, polyolefin, polyurethane, polyester, polyamide, polybutadiene, ethylene-vinyl acetate copolymer, polyvinyl chloride, natural rubber, fluororubber, polyisoprene, chlorinated polyethylene, styrene-butadiene rubber, silicone rubber and so on.

As for the proportion of a thermoplastic elastomer to the whole binder, the range of 10 to 100 wt % serves the purpose. However, it is preferable for the thermoplastic elastomer to constitute the highest possible percentage of the binder, especially 100 wt % of the binder.

Suitable examples of a solvent which can be used for preparing the coating composition include lower alcohols such as methanol, ethanol, n-propanol, n-butanol, etc.; chlorine-containing hydrocarbons such as methylene chloride, ethylene chloride, etc.; ketones such as acetone, methyl ethyl ketone, methyl isobutyl ketone, etc.; esters prepared from lower alcohols and lower fatty acids, such as methyl acetate, ethyl acetate, butyl acetate, etc.; ethers such as dioxane, ethylene glycol monoethyl ether, ethylene glycol monomethyl ether, etc.; and mixtures of two or more of the above-cited solvents.

A proper ratio between a binder and a phosphor in the coating composition depends on the characteristics required of the radiation intensifying screen to be made and the type of the phosphor. In general, however, the ratio between the binder and the phosphor is chosen from the range of 1:1 to 1:100 by weight, and particularly preferably from the range of 1:8 to 1:40 by weight.

In the coating composition, there may be added various additives including a dispersing agent for improving upon the dispersibility of the phosphor in the coating composition and a plasticizer for heightening the bonding strength between the binder and the phosphor in the phosphor layer formed. Specific examples of a dispersing agent used for the foregoing purpose include phthalic acid, stearic acid, caproic acid and oleophilic surfactants, and those of a plasticizer include phosphoric acid esters such as triphenyl phosphate, tricresyl phosphate, diphenyl phosphate, etc.; phthalic acid esters such as diethyl phthalate, dimethoxyethyl phthalate, etc.; glycolic acid esters such as ethyl phthalylethyl glycolate, butyl phthalylbutyl glycolate, etc.; and polyesters prepared from polyethylene glycol and aliphatic dibasic acids, such as polyester prepared from triethylene glycol and adipic acid, polyester prepared from diethylene glycol and succinic acid, etc.

The thus prepared coating composition containing the phosphor and the binder is then coated uniformly on the surface of a temporary support for sheet formation use. This coating operation can be carried out using a doctor blade, a roll coater, a knife coater or the like.

The temporary support can be arbitrarily chosen, e.g., from a glass plate, a metal plate and materials known to be usable as the support of radiation intensifying screens. Specific examples of a material for the temporary support

include plastic films such as cellulose acetate film, polyester film, polyethylene terephthalate film, polyamide film, polyimide film, triacetate film, polycarbonate film, etc.; metal sheets such as aluminum foil, aluminum alloy foil, etc.; plain paper, baryta paper, resin-coated paper, pigment paper in which a pigment such as titanium oxide is incorporated, paper sized with polyvinyl alcohol or the like; and plates or sheets of ceramics, such as alumina, zirconia, magnesia, titania, etc.

The coating composition for formation of the phosphor layer is coated on the temporary support, dried and then peeled off the temporary support. Thus, a phosphor sheet to constitute the phosphor layer of a radiation intensifying screen is obtained. Accordingly, it is desirable that a surface lubricant be applied in advance to the surface of the temporary support, thereby making it easy to peel the phosphor sheet off the temporary support.

Then, the step (b) is described in detail.

Firstly, a support is arranged for the phosphor sheet formed in the above-described manner. This support can be chosen arbitrarily from the same materials as used in forming a phosphor sheet.

In preparing conventional radiation intensifying screens, it is known to apply a high molecular substance, such as gelatin, to a support as an adhesion providing layer on the side where a phosphor layer is to be provided for the purpose of strengthening the binding of a phosphor layer to a support, or to coat the surface of a support, on which a phosphor layer is to be provided, with a light reflecting layer containing a light reflecting substance such as titanium oxide or with a light absorbing layer containing a light absorbing substance such as carbon black in order to improve upon the sensitivity or the image qualities (sharpness, graininess) as radiation intensifying screen. Also on the support used in the present invention, those layers can be coated, and how to constitute and combine them can be properly chosen depending upon the purpose in using the radiation intensifying screen in the present invention.

The phosphor sheet obtained in the step (a) is superposed on a support, and then compressively stressed at a temperature higher than the softening or melting point of the binder used therein, thereby making the phosphor sheet adhere to the support.

By adopting the method of compressively stressing the phosphor sheet on the support without previous fixation, as in the above-described manner, the sheet can be spread out into a thinner sheet, the phosphor therein can be inhibited from suffering damage, and a higher packing rate of the phosphor can be achieved under the same pressure applied to the sheet in comparison with the case in which the sheet is pressed as it is fixed to the support. As for the device used in the present invention for the compressive stressing treatment, conventionally used devices such as a calender roll, a hot press and so on are suitable examples thereof. Specifically, the compressive stressing treatment using a calender roll is carried out by superposing the phosphor sheet obtained in the step (a) on the support and passing them at a constant speed between a pair of rollers heated up to a temperature higher than the softening or melting point of the binder. As for the compressive stressing device, those usable in the present invention should not be construed as being limited to the above-cited ones, but any devices which enable the compressive stressing of the sheet under heating can be used in the present invention.

Upon compressive stressing, it is desirable that the pressure of at least 50 kgw/cm<sup>2</sup> be imposed on the sheet.

In conventional radiation intensifying screens, a transpar-

ent protective film is provided on the surface of the phosphor layer, the reverse side of which is contact with the support, for the purpose of protecting the phosphor layer physically and chemically. Also in the radiation intensifying screen used in the present invention, it is desirable to coat the phosphor layer with such a transparent protective film.

The thickness of the protective film is generally in the range of about 0.1  $\mu\text{m}$  to about 20  $\mu\text{m}$ .

The transparent protective film can be provided on the surface of the phosphor layer by coating the phosphor layer with a solution prepared by dissolving in an appropriate solvent a transparent high molecular substance such as a cellulose derivative (e.g., cellulose acetate, cellulose nitrate) or a synthetic polymer (e.g., polymethylmethacrylate, polyvinyl butyral, polyvinyl formal, polycarbonate, polyvinyl acetate, vinyl chloride-vinyl acetate copolymers). The protective film can also be provided in another manner such that a protective film forming sheet, e.g., a plastic sheet such as a sheet of polyethylene terephthalate, polyethylene naphthalate, polyethylene, polyvinylidene chloride, polyamide, etc., or a transparent glass plate, is prepared in advance, and then bonded to the surface of the phosphor layer using an appropriate adhesive.

As for the protective film of the radiation intensifying screen used in the present invention, a film formed from a coating composition containing an organic solvent-soluble fluororesin is preferred in particular. The term "fluororesin" as used herein is intended to include homopolymers of fluorine-containing olefins (fluoroolefins) and copolymers containing fluorine-containing olefins as a copolymerizing component. A film as a fluororesin coating may undergo a cross-linking reaction. The protective film of a fluororesin has advantages in that stains such as a plasticizer and other additives oozed out of an X-ray film or the like are hard to permeate into the protective film even when these films are brought into contact with each other, so that the stains can be easily removed, e.g., by wiping them off.

Also in the case using an organic solvent-soluble fluororesin as protective film forming material, film formation can be easily performed by coating a solution prepared by dissolving a fluororesin in an appropriate solvent and then by drying it. More specifically, a coating solution containing an organic solvent-soluble fluororesin as a protective film forming material is uniformly applied to the surface of the phosphor layer with a doctor blade or the like and then dried to make it into a film. The protective film and the phosphor layer may be formed at the same time using a simultaneous double-layered coating technique.

Specific examples of the foregoing fluororesin, which is, as described above, a homopolymer of fluorine-containing olefin (a fluoroolefin homopolymer) or a copolymer containing a fluoroolefin as a copolymerizing component, include polytetrafluoroethylene, polychlorotrifluoroethylene, polyvinyl fluoride, polyvinylidene fluoride, tetrafluoroethylene-hexafluoropropylene copolymers and fluoroolefine-vinyl ether copolymers. Although fluororesins are generally insoluble in organic solvents, the copolymers containing fluoroolefins as a copolymerizing component can be rendered soluble in organic solvents by other constitutional units (a copolymerizing component other than fluoroolefins). Therefore, a coating solution can be easily prepared by dissolving such copolymers in an appropriate solvent, and it can be easily made into a film by coating it on the phosphor layer and then drying it. As for the copolymer described above, fluoroolefin-vinyl ether copolymers are examples thereof. In addition, polytetrafluoroethylene and modification products thereof are soluble in certain

fluorine-containing organic solvents, e.g., perfluoro solvents. Therefore, in analogy with the foregoing copolymers containing fluoroolefins as copolymerizing component, those polymers also can be made into a protective film using a coating technique.

In the protective film, a resin other than a fluororesin may be contained, and a cross-linking agent, a hardening agent, a yellowing inhibitor and so on may also be contained. For fully achieving the above-described purpose, however, it is desirable to control the content of a fluororesin in the protective film to at least 30 wt %, preferably at least 50 wt %, and particularly preferably at least 70 wt %. Specific examples of a resin which can be contained in the protective film in addition to a fluororesin include polyurethane resins, polyacrylic resins, cellulose derivatives, polymethylmethacrylate, polyester resins, epoxy resins and so on.

Further, the protective film of the intensifying screen used in the present invention may be a coating in which either an oligomer having a polysiloxane skeleton or an oligomer containing perfluoroalkyl groups, or both of them are contained. As for the oligomer having a polysiloxane skeleton, an oligomer having a dimethylpolysiloxane skeleton is an example thereof, and it is desirable that the oligomer has at least one functional group (e.g., hydroxyl group). Further, it is favorable for the oligomer to have a weight-average molecular weight of from 500 to 100,000, preferably from 1,000 to 100,000, and particularly preferably from 3,000 to 10,000. As for the oligomer containing perfluoroalkyl groups, on the other hand, it is desirable that the oligomers contain at least one functional group (e.g., hydroxyl group) in a molecule, and has a weight-average molecular weight of from 500 to 100,000 (on weight average), preferably from 1,000 to 100,000, and particularly preferably from 10,000 to 100,000. The oligomer containing a functional group is used to advantage. This is because the effect produced by addition of the oligomer can last long since a cross-linking reaction takes place between the functional group of the oligomer and a protective film-forming resin upon formation of the protective film, and thereby the oligomer is introduced into the molecular structure of the film-forming resin. Owing to the introduction of the oligomer into the resin molecule, it does not occur that the oligomer is removed from the protective film by long-term repeated use of the radiation-image transforming panel, a cleaning operation for the protective film surface or so on.

In the protective film, it is desirable that the oligomer is contained in a proportion of 0.01 to 10 wt %, particularly 0.1 to 2 wt %.

Furthermore, the protective film may contain a perfluoroolefin resin powder or a silicone resin powder. The perfluoroolefin resin powder and the silicone resin powder are preferably have their respective average grain sizes in the range of 0.1 to 10  $\mu\text{m}$ , particularly 0.3 to 5  $\mu\text{m}$ . Such a powder is desirably contained in the protective film in a proportion of 0.5 to 30 wt %, preferably 2 to 20 wt %, and particularly preferably 5 to 15 wt %, to the whole weight of the protective film.

As described above, it is desirable that the radiation intensifying screen used in the present invention be designed so as to have high sensitivity and to bear characteristics such that the contrast transfer function (CTF) values are at least 0.79 at the spacial frequency of 1 line/mm (1 p/mm) and at least 0.36 at the spacial frequency of 3 lines/mm (3 p/mm).

Further, when a graph is drawn, with spacial frequency (line number/mm) as abscissa and contrast transfer function (CTF) as ordinate, by successively connecting the points represented by the following data on the relation between

the line number/mm and CTF values so as to form a smooth curve, it is especially desirable that the radiation intensifying screen used in the present invention have as its characteristics higher CTF values than the CTF values on the aforementioned curve over the whole range of spacial frequency.

| line(s)/mm | CTF   |
|------------|-------|
| 0.00       | 1.00  |
| 0.25       | 0.950 |
| 0.50       | 0.905 |
| 0.75       | 0.840 |
| 1.00       | 0.790 |
| 1.25       | 0.720 |
| 1.50       | 0.655 |
| 1.75       | 0.595 |
| 2.00       | 0.535 |
| 2.50       | 0.430 |
| 3.00       | 0.360 |
| 3.50       | 0.300 |
| 4.00       | 0.255 |
| 5.00       | 0.180 |
| 6.00       | 0.130 |

The measurement and the calculation of the contrast transfer function from the radiation intensifying screen to the photosensitive material can be carried out using the sample obtained by printing a rectangular chart on a one-sided material MRE, products for mammography of Eastman Kodak Co.

The radiation intensifying screens suitable for the present invention, which have the characteristics illustrated above, can be obtained, e.g., by using as binder such thermoplastic elastomers as described above, and adopting a method comprising a step of compressively stressing the phosphor layer.

The protective layer of the radiation intensifying screen is preferably a transparent synthetic resin layer having a thickness of 5  $\mu\text{m}$  or less which is formed on a phosphor layer using a coating technique. Such a thin protective layer can diminish the distance from the phosphor in the radiation intensifying screen to the silver halide photographic material, and so it can contribute to improvement in sharpness of the X-ray image formed in the photographic material.

In recent years, a high-temperature rapid development processing has been rapidly spread into the photosensitive materials, and in automatic development processing of various photosensitive materials, the processing time has greatly been reduced.

In particular, in X-ray photosensitive materials for direct radiography, there is a competition in the processing time and rapid processing systems which enables 45 seconds' dry-to-dry processing have been marketed. On carrying out urgent medical diagnosis, it is very important to subject X-ray photosensitive materials to rapid development processing. Therefore, the demand for rapid processing has been increased. In order to attain this rapid processing system, it is necessary to keep the photographic performance and disolor the sensitizing dye and/or the crossover cut dye with the short developing time.

As for the image-forming system of the present invention, it is desirable that the silver halide photographic material, which has on the front and the back sides respectively the light-sensitive layers fulfilling the aforementioned sensitivity requirements and bearing characteristics substantially the same in both layers, be combined with the radiation intensifying screens having characteristics as defined above, and that substantially the same in both screens, so that the screens may be disposed on both sides (the front and the

back sides) of the photographic material respectively. However, as disclosed in U.S. Pat. No. 4,710,637, the intensifying screen on the front side may be lower in phosphor content than the intensifying screen on the back side in order to acquire improved balance between the image sharpness and the photographic speed.

More specifically, in order that the system of the present invention has such a degree of photographic speed as not to cause problems in practical use and ensures a high level of quality to the X-ray image formed therein by photograph-taking, it is desirable that the silver halide photographic material be combined with two sheets of radiation intensifying screens so that the resulting system may achieve such photographic speed that the image having a density of 1.0 can be formed when the system is exposed to 0.5–1.5 mR of X rays emitted from a 80 KVp three-phase X-ray source and the development-processing is carried out with the developer defined hereinbefore under the condition also defined hereinbefore.

For evaluation of the system constituted of the present silver halide photographic material and two sheets of radiation intensifying screens, the following determination method is adopted. The basis of the evaluation is also described below.

As a generally used method for determining the image efficiency of the X-ray photograph taking system which is constituted of a silver halide photographic material and radiation intensifying screens, there is a method of determining the quantum detecting efficiency (DQE). On the other hand, there is the determination of noise equivalent quantum (NEQ) as the method of measuring the image by collectively evaluating sharpness and granularity. DQE is the quotient of the  $(\text{signal/noise})^2$  value of the image, which is finally formed in the photographic material by the X-ray photography using the foregoing system, divided by the  $(\text{signal/noise})^2$  value of the incident X rays. While DQE becomes 1 in a case that ideal image formation is performed, it is less than 1 in usual cases. On the other hand, NEQ is the numerical value corresponding to  $(\text{signal/noise})^2$  of the final image. Further, there is the following relationship between DQE and NEQ:

$$\text{DQE}(\nu) = \text{NEQ}(\nu)/Q$$

$$\text{NEQ}(\nu) = (\log_{10} \text{exy}(\text{MTF}(\nu))^2 / \text{NPS}_0(\nu))$$

wherein  $\gamma$  is contrast,  $\text{MTF}(\nu)$  is the modulation transfer function of an image,  $\text{NPS}_0(\nu)$  is the power spectrum of output noise,  $\nu$  is a spacial frequency, and  $Q$  is an incident X-ray quantum number.

The relationship between the photographic speed and the image quality can be evaluated using DQE. Specifically, a high DQE value system suggests that the system is excellent in balance between the photographic speed and the image quality. On the other hand, the image quality of the final image can be evaluated using NEQ. Specifically, the higher the NEQ value is, the better quality the image can be judged to have. However, NEQ is a value referring to the evaluation of physical image quality, but it does not always have one-to-one correspondence to clinical image discrimination. Because if there is a great difference between the granularity and the sharpness of the image, it cannot be said that the image provides a high visible image quality clinically. In evaluating the image quality from the clinical point of view, it is therefore desirable to use both NEQ and MTF values.

## [1] Preparation of High-Speed Tabular-Grain Emulsions A, B and C

One liter of water, 6.9 g of potassium bromide and 9.5 g of low molecular weight gelatin (average molecular weight: 15,000) were placed in a vessel and kept at 55° C. Thereto, 37 ml of a water solution containing 2.4 g of silver nitrate and 38 ml of water solution containing 5.9 g of potassium bromide were added over a 37-second period with stirring in accordance with a double jet method. Then, 18.6 g of gelatin was further added thereto. The resulting reaction mixture was heated up to 70° C. and thereto, 100 ml of a water solution containing 11.2 g of silver nitrate was added over a 22-minute period. Then, 8.5 ml of 25% aqueous ammonia was added thereto, and stood for 10 minutes under the temperature kept as it was, thereby carrying out physical ripening. Thereafter, 8 ml of 100% acetic acid was added thereto. Subsequently, in accordance with a controlled double jet method, a water solution containing 145 g of silver nitrate and a water solution containing potassium bromide were added at an accelerated flow rate (initial flow rate/final flow rate=1/5.4) over a 35-minute period as the pAg of the reaction system was maintained at 8.5. Then, 35 ml of a 2N solution of potassium thiocyanate was added thereto. The thus obtained emulsion was physically ripened by 5-minute standing under the temperature unchanged. Thereafter, the temperature of the emulsion was lowered to 35° C. Thus, there were obtained tabular grains of pure silver bromide having an average diameter of 1.25 μm, on a projection area basis, a thickness of 0.18 μm and a variation coefficient of 20% with respect to the diameter.

Then, the water-soluble salts were removed from the physically ripened emulsion by a flocculation method. The resulting emulsion was warmed again to 40° C. admixed with 35 g of gelatin, 2.35 g of phenoxyethanol and 0.8 g of sodium polystyrenesulfonate as a thickener, and further adjusted to pH 5.9 and pAg 8.00 using sodium hydroxide and a silver nitrate solution.

The emulsion thus obtained was chemically sensitized as it was kept at 56° C. with agitating. Specifically, in order to effect the chemical sensitization, the emulsion was admixed with successive,  $1 \times 10^{-5}$  mole/mole Ag of  $C_2H_5SO_2Sn$ , 0.1 mol % of fine-grained AgI, 480 mg of Sensitizing Dye I, 0.83 g of calcium chloride, 0.9 mg of sodium thiosulfate, 1.9 mg of Selenium Compound I, 1.9 mg of chloroauric acid and 90 mg of potassium thiocyanate, and then allowed to stand for 40 minutes. Thereafter, the resulting emulsion was cooled to 35° C.

Thus, the preparation of a tabular-grain emulsion was completed. The thus prepared tabular-grain emulsion was named Emulsion A.



-continued

## Selenium Compound I



In addition, tabular-grain Emulsions B and C were prepared in the same manner as Emulsion A, except that the preparation condition was changed to those shown in Table 1 respectively. The thus prepared Emulsions A, B and C were different in average projection area diameter from one another.

TABLE 1

|                                             | Emulsion A      | Emulsion B      | Emulsion C      |
|---------------------------------------------|-----------------|-----------------|-----------------|
| Preparation temp.                           | 55° C. → 70° C. | 60° C. → 75° C. | 55° C. → 70° C. |
| Amount of low molecular weight gelatin used | 9.5 g           | 9.5 g           | 7 g             |
| Average projection area diameter            | 1.25 μm         | 1.50 μm         | 1.05 μm         |

## [2] Preparation of Fine-Grain Hard-Gradation Emulsions D, E and F

To one liter of a 2 wt % of gelatin solution containing 5.3 g of potassium bromide and 4 g of sodium p-toluenesulfonate, 10 mg of sodium thiosulfate pentahydrate, 1.4 g of potassium thiocyanate and 10 ml of glacial acetic acid were added. To the resulting mixture under vigorous agitation, 14 ml of a water solution containing 5.2 g of silver nitrate and 7 ml of a water solution containing 1.8 g of potassium bromide and 0.33 g of potassium iodide were added for 30 seconds in accordance with a double jet method. Thereafter, 30 ml of a water solution containing 3 g of potassium iodide was further added thereto.

Furthermore to the resulting mixture, 200 ml of a water solution containing 78 g of silver nitrate was added over a 15-minute period and then, after an interval of one minute, 200 ml of a water solution containing 50.6 g of potassium bromide and 3.65 g of potassium iodide was added over a 15-minute period. Next, the reaction mixture was admixed with 14 ml of 25 wt % aqueous ammonia, and ripened for 10 minutes. Thereto, a water solution containing 117 g of silver nitrate and a water solution containing 82.3 g of potassium bromide were simultaneously added over a 14-minute period. The temperature of the reaction system in the whole preparation process was kept at 70° C.

The foregoing reaction solution was washed in a conventional manner, that is, using a flocculation method, and then admixed with gelatin, a thickener and antiseptics at 40° C. to prepare a dispersion. After the dispersion was adjusted to pH 5.6 and pAg 8.9, it was admixed with 21 mg of 4-hydroxy-6-methyl-1,3,3a,7-tetraazaindene and 460 mg of Sensitizing Dye I as it was maintained at 55° C. After 10 minutes' ripening, the resulting mixture was further admixed with successive, 3.8 mg of sodium thiosulfate pentahydrate, 3.8 mg of Selenium Compound II, 77 mg of

potassium thiocyanate and 2.6 mg of chloroauric acid, and ripened again for 50 minutes. Then, it was admixed with 70 mg of 4-hydroxy- 6-methyl-1,3,3a,7-tetrazaindene, and cooled. Thus, fine-grain monodisperse non-tabular grain Emulsion D was obtained.



In addition, monodisperse fine-grain Emulsions E and F were prepared in the same manner as Emulsion D, except that the preparation condition was changed to those shown in Table 2. Thus, Emulsions D, E and F different in average grain size were obtained.

TABLE 2

|                                                         | Emulsion D | Emulsion E | Emulsion F |
|---------------------------------------------------------|------------|------------|------------|
| Amount of potassium thiocyanate added                   | 1.4 g      | 4.0 g      | 1.0 g      |
| Average sphere-corresponding diameter ( $\mu\text{m}$ ) | 0.46       | 0.68       | 0.40       |
| Variation coefficient (%)                               | 17         | 20         | 15         |

### [3] Preparation of Supports X, Y and Z

#### (1) Preparation of Dye Dispersion A for Subbing Layer

The following Dye-I was treated with a ball mill according to the method disclosed in JP-A-63-197943.



Water in an amount of 434 ml and 791 ml of a 6.7% water solution of a surfactant, Triton X-200, were placed in a 2-liter ball mill. Thereto, 20 g of Dye-I and 400 ml of zirconium oxide ( $\text{ZrO}_2$ ) beads (2 mm in diameter) were added successively. The content in the ball mill was ground for 4 days. Then, 160 g of 12.5% gelatin solution was added thereto. After defoaming, the  $\text{ZrO}_2$  beads were filtered out. According to the observation of the thus obtained dye dispersion, the ground dye had a wide particle size distribution. More specifically, the diameters of the dye particles are in the range of 0.05 to 1.15  $\mu\text{m}$  and an average particle size thereof was 0.37  $\mu\text{m}$ .

From the dispersion, dye particles measuring no smaller than 0.9  $\mu\text{m}$  in size were removed by a centrifuging operation. Thus, Dye Dispersion A was obtained.

#### (2) Preparation of Support

A biaxially stretched 175  $\mu\text{m}$ -thick blue-colored polyethylene terephthalate film was subjected to a corona discharge treatment, and then coated with 4.9  $\text{ml}/\text{m}^2$  of a first subbing layer having the following composition by means of a wire-bar coater, and dried at 185° C. for 1 minutes.

On the back side also, the first subbing layer was provided in the same manner as described above.

10

| Composition of First Subbing Layer |                                                                                                               |        |
|------------------------------------|---------------------------------------------------------------------------------------------------------------|--------|
|                                    | Butadiene-styrene copolymer latex solution (solid proportion: 40%, butadiene/styrene ratio = 31/69 by weight) | 158 ml |
| 15                                 | Sodium 2,4-dichloro-6-hydroxy-s-triazine (4% solution)                                                        | 41 ml  |
|                                    | distilled water                                                                                               | 300 ml |

20

The first subbing layer on each side of the film was coated with the second subbing layer having the following composition by means of a wire-bar coater and dried at 155° C. so that the following ingredients might have their respective coverage rates set forth below.

25

| Composition of Second Subbing Layer |                                                                                               |                             |
|-------------------------------------|-----------------------------------------------------------------------------------------------|-----------------------------|
|                                     | Gelatin                                                                                       | 160 $\text{mg}/\text{m}^2$  |
| 30                                  | Dye Dispersion A (on a solids basis)                                                          | 25 $\text{mg}/\text{m}^2$   |
|                                     | $\text{C}_{12}\text{H}_{25}\text{O} (\text{CH}_2\text{CH}_2\text{O})_{10}\text{H}$            | 1.8 $\text{mg}/\text{m}^2$  |
|                                     | Proxel                                                                                        | 0.27 $\text{mg}/\text{m}^2$ |
|                                     | Matting agent (polymethylmethacrylate particles having an average size of 2.5 $\mu\text{m}$ ) | 2.5 $\text{mg}/\text{m}^2$  |

35

Thus, Support X containing a crossover cut layer was prepared. In addition, Supports Y and Z were prepared in the same manner as Support X, except that the preparation condition was changed to those shown in Table 3.

40

TABLE 3

|    | Support X                                       | Support Y | Support Z |      |
|----|-------------------------------------------------|-----------|-----------|------|
| 45 | Coverage of Dye-I ( $\text{mg}/\text{m}^2$ )    | 25        | 0         | 40   |
|    | Undercoat thickness (upper layer) $\mu\text{m}$ | 0.17      | 0.15      | 0.16 |
|    | Density (both-side) at 550 nm                   | 0.48      | 0.12      | 0.70 |

50

### [4] Preparation of Coating Composition

To each of tabular-grain Emulsions A to C, the following ingredients were added to prepare a coating composition for the upper emulsion layer. On the other hand, the ingredients described below were added to each of fine-grain monodisperse Emulsions D to F to prepare a coating composition for the lower emulsion layer. In addition, the coating composition for a protective layer was prepared.

60

#### Coating Composition for Upper Emulsion Layer:

|                                                                                      |                                |
|--------------------------------------------------------------------------------------|--------------------------------|
| Emulsion A, B or C                                                                   | 1 Kg (gelatin: 41 g, Ag: 94 g) |
| Polymer latex (ethylacrylate/methacrylic acid ratio in the polymer = 97/3 by weight) | 24.4 g                         |

-continued

## Coating Composition for Upper Emulsion Layer:

Hardener [1,2-bis(vinylsulfonylacetamido)ethane] 3.4 g  
 2,6-Bis(hydroxyamino)-4-diethylamino-1,3,5-triazine 0.13 g  
 Sodium polystyrenesulfonate (average molecular weight: 600,000) 5.3 g  
 Dextran (average molecular weight: 39,000) 28 g  
 Gelatin gel (on a solid basis) 61 g  
 Gelatin gel (on a solid basis) 4.8 g



## Coating Composition for Lower Emulsion Layer:

Emulsion D, E or F 1 Kg (gelatin: 83 g, Ag: 92 g)  
 Dextran (average molecular weight: 39,000) 18 g  
 Sodium polyacrylate (average molecular weight: 41,000) 3 g  
 Sodium polystyrenesulfonate (average molecular weight: 600,000) 1 g  
 Potassium iodide 50  
 Trimethylol propane 83 mg  
 Polymer latex (ethylacrylate/methacrylic acid ratio in the polymer = 97/3 by weight) 5 g  
 Hardener [1,2-bis(vinylsulfonylacetamido)ethane] 5 g  
 2,6-Bis(hydroxyamino)-4-diethylamino-1,3,5-triazine 2.7 g  
 55



-continued

## Coating Composition for Lower Emulsion Layer:

70 mg

5

10

15

20

25

30

0.4 g

12.6 mg

35

up to 4 liter

40

10 mg

Distilled Water up to 2.2 l

Dye Emulsion

Dye

Chemical structures for the Dye Emulsion and Dye components are shown. The Dye Emulsion structure is a benzene ring with a -SO3Na group and a -N=N-CH2-CH2-SH group attached. The Dye structure is a trisubstituted benzene ring with two -NH-C6H4-C2H5 groups and one -NH-C6H4-C2H5 group attached.

## Coating Composition for Protective Layer:

1 kg

200 g

39 9

1.6 g

7 g

91 g

0.7 g

45 g

3 g

1.6 g

24 g

14.4 l

Gelatin

Dextran (average molecular weight: 39,000)

C<sub>16</sub>H<sub>33</sub>O(CH<sub>2</sub>CH<sub>2</sub>O)<sub>10</sub>H

C<sub>8</sub>F<sub>17</sub>SO<sub>2</sub>N(C<sub>3</sub>H<sub>7</sub>)(CH<sub>2</sub>CH<sub>2</sub>O)<sub>4</sub>(CH<sub>2</sub>)SO<sub>3</sub>Na

C<sub>8</sub>F<sub>17</sub>SO<sub>3</sub>K

Polymethylmethacrylate particles (average particle size: 3.7  $\mu$ m)

Proxel

Sodium polyacrylate (average molecular weight: 41,000)

Sodium polystyrenesulfonate (average molecular weight: 600,000)

NaOH

C<sub>8</sub>H<sub>17</sub>C<sub>6</sub>H<sub>4</sub>(OCH<sub>2</sub>CH<sub>2</sub>)<sub>3</sub>SO<sub>3</sub>Na

Distilled water up to 10

## [5] Preparation of Photosensitive Materials

Each photosensitive material was prepared under the same condition by coating and drying the coating compositions prepared in [4] on both sides of the support prepared in [3] in accordance with a simultaneous extrusion method. Therein, the gelatin coverage of the protective layer was adjusted to 1 g/m<sup>2</sup>. The coating conditions are summarized in Table 4.

TABLE 4

| Sample No. | Upper Emulsion (Ag amount*: g/m <sup>2</sup> ) | Lower Emulsion (Ag amount*: g/m <sup>2</sup> ) | Support (dye amount*: mg/m <sup>2</sup> ) | Note       |
|------------|------------------------------------------------|------------------------------------------------|-------------------------------------------|------------|
| 1          | Emulsion A (1.7)                               | —                                              | X (25)                                    | comparison |
| 2          | Emulsion B (1.7)                               | —                                              | X (25)                                    | comparison |
| 3          | Emulsion C (1.7)                               | —                                              | X (25)                                    | comparison |
| 4          | Emulsion D (1.7)                               | —                                              | X (25)                                    | comparison |
| 5          | Emulsion E (1.7)                               | —                                              | X (25)                                    | comparison |
| 6          | Emulsion F (1.7)                               | —                                              | X (25)                                    | comparison |
| 7          | Emulsion A (0.16)                              | Emulsion D (1.5)                               | X (25)                                    | invention  |
| 8          | Emulsion A (0.22)                              | Emulsion D (1.5)                               | X (25)                                    | invention  |
| 9          | Emulsion A (0.30)                              | Emulsion D (1.5)                               | X (25)                                    | invention  |
| 10         | Emulsion A (0.40)                              | Emulsion D (1.2)                               | X (25)                                    | comparison |
| 11         | Emulsion A (0.60)                              | Emulsion D (1.0)                               | X (25)                                    | comparison |
| 12         | Emulsion A (0.22)                              | Emulsion D (1.5)                               | Y (0)                                     | comparison |
| 13         | Emulsion A (0.22)                              | Emulsion D (1.5)                               | Z (40)                                    | invention  |
| 14         | Emulsion B (0.26)                              | Emulsion E (1.7)                               | X (25)                                    | invention  |
| 15         | Emulsion B (0.36)                              | Emulsion E (1.7)                               | X (25)                                    | invention  |
| 16         | Emulsion B (0.46)                              | Emulsion E (1.5)                               | X (25)                                    | comparison |
| 17         | Emulsion B (0.26)                              | Emulsion E (1.7)                               | Y (0)                                     | comparison |
| 18         | Emulsion B (0.26)                              | Emulsion E (1.7)                               | Z (40)                                    | invention  |
| 19         | Emulsion C (0.20)                              | Emulsion F (1.4)                               | X (25)                                    | invention  |
| 20         | Emulsion C (0.20)                              | Emulsion F (1.4)                               | Y (0)                                     | comparison |
| 21         | Emulsion C (0.20)                              | Emulsion F (1.4)                               | Z (40)                                    | invention  |

\*The values shown in parenthesis mean the coated amount per one side.

25

### [6] Sensitometry

Each of the photosensitive materials as subjects of evaluation was sandwiched between two sheets of commercial screen, HR-4, products of Fuji Photo Film Co., Ltd., and subjected to stepwise exposure in which the amount of X rays was changed by a width of  $\log E=0.15$  at a step in accordance with a distance method.

Therein, there was used an X-ray tube, DRX-3724 HD, products of Toshiba Electric Co., Ltd., which emitted X rays using a tungsten target and setting its focal spot size at 0.6 mm $\times$ 0.6 mm via an iris and 3 mm-thick aluminum equivalent material. The X rays emitted by applying an electric potential of 80 KVp to the X-ray tube with a three-phase pulse generator was passed through a filter of 7 cm-thick water having absorption almost equivalent to the human body. The resulting X rays were used herein as the light source.

After photographing, each photosensitive material was subjected to the photographic processing operation described hereinbefore using a roller conveyable type automatic developing machine (Auto Processor Model FPM-5000, made by Fuji Photo Film Co., Ltd.), wherein the development-processing was carried out at 35° C. using Developer I and the fixation-processing at 25° C. using Fixer F (comprising 200 ml of ammonium thiosulfate (70% by weight/volume), 20 g of sodium sulfite, 8 g of boric acid, 0.1 g of disodium ethylenediaminetetraacetate (dihydrate), 15 g of aluminum sulfate, 2 g of sulfuric acid, 22 g of glacial acetic acid and water in such an amount as to make the total volume one liter, and being adjusted to pH 4.5), thereby obtaining a sample for measurement.

The density measurement of the thus obtained samples was carried out with visible rays, and the characteristic curves thereof were determined.

The reciprocal of the exposure amount of X rays required for providing the density of 1.8 was taken as the standard of sensitivity. The sensitivities of the samples were shown as relative values. Moreover, the characteristic curves obtained were each differentiated to determine gamma values, thereby plotting the obtained data, with the gamma value as ordinate and  $\log E$  as abscissa. Using the thus obtained

gamma curve, point gamma values corresponding to the density range of 1.6 to 2.0 were determined. In addition, there was determined the point gamma value corresponding to the exposure amount reduced to  $1/10$  the exposure amount required for providing the density of 1.8. The results obtained are shown in Table 5. Additionally, the slope of the straight line connecting the two points corresponding to the density 1.6 and the density 2.0 on each characteristic curve was determined, which is also shown in Table 5 as average gradient.

### [7] Determination of Crossover Rate

Each silver halide photographic material was inserted between a radiation intensifying screen, HR-4 (which uses a terbium-activated gadolinium oxysulfide phosphor (main wavelength of emission: 545 nm, green light), and a sheet of black paper, and irradiated with X rays from the black paper side. The X-ray source used herein was the same source as used in the sensitometry described above. In the irradiation, the amount of X rays was changed by a distance method. After the irradiation, the photographic material was subjected to the same photographic processing operation as in the sensitivity measurement described above. The thus processed photographic material was divided into two pieces. The light-sensitive layer on one side was delaminated from one piece, and that on the other side from the other piece. The density of the light-sensitive layer on the side with which the intensifying screen had been in contact was higher than the density of the light-sensitive layer disposed on the reverse side. There were respectively depicted characteristic curves of the foregoing two light-sensitive layers, and determined the average difference in sensitivity ( $\Delta \log E$ ) between the respective straight line portions (the density range of 0.5 to 1.0) of the two characteristic curves. Thus, the crossover rate was calculated using this average value and the following equation:

$$\text{Crossover Rate (\%)} = 100 / (\text{antilog}(\Delta \log E) + 1)$$

## [8] Determination of CTF

Each of the photosensitive materials as subjects of evaluation was sandwiched between two sheets of Screen HR-4, and placed at a distance of 2 m from an X-ray source. The X-ray source used was the same as used in the foregoing sensitometry. A photograph of a rectangular chart for MTF measurement (made of molybdenum, having a thickness of 80  $\mu$ m and spacial frequencies from 0 line/mm to 10 lines/mm) was taken using the foregoing X-ray image forming system. The photographic processing condition adopted therein was the same as in the foregoing sensitometry.

As for the exposure amount, it was controlled by changing the exposure time of X-rays so that the area corresponding to the molybdenum-unshielded part might have a density of 1.8.

Each of the X-ray photograph samples was scanned with a microdensitometer. The aperture used therein was a slit 30  $\mu$ m wide in the scanning direction and 500  $\mu$ m wide in the direction perpendicular to the scanning direction, and the density profile of each sample was determined at sampling intervals of 30  $\mu$ m. This scanning operation was repeated 20 times, thereby calculating the average. The thus obtained average was taken as the density profile forming the basis of CTF calculation. Then, a square wave peak was detected at every frequency in the density profile, and thereby was calculated the density contrast at every frequency.

The density contrast values at the spacial frequencies 1 line/mm and 3 lines/mm are shown in Table 5.

of 140 cm. The X-ray source was equipped with a 3 mm-thick aluminum equivalent filter, had a focal spot size of 0.6 mm  $\times$  0.6 mm and emitted X rays under the potential of 100 KVp (three-phase 12-pulse).

In analogy with the case in which the photographic characteristics were examined, the photographic processing of each photosensitive material was carried out at 35°C. for 90 seconds (development time: 25 seconds) using an automatic developing machine, FPM-5000, Developer RDIII having the same composition as that of Developer I described above and Fixer F described above.

The exposure amount of X rays was controlled by changing the exposure time so that it could provide the density of 1.8 at one point chosen in the lung field. The finished photograph of the thorax phantom was put on a Schaukasten, and the evaluation thereof was made by visual observation. Specifically, each photograph was examined as to whether the shadow of blood vessels in the lung field and the organs in the mediastinum were seen easily. The case they were seen definitely was graded A, the case they were seen well was graded B, the case they were seen to such an extent as to enable a bare diagnosis was graded C, and the case the diagnosis was impossible was graded D. When there was significant difference in easiness of seeing among photograph samples even when the same grade was given thereto, a or z was added to the grading mark, such as Aa (superior to other photographs graded A), Az (inferior to other photographs graded A), or the like. The results obtained are shown in Table 5.

TABLE 5

| Sam-<br>ple<br>No. | Sensi-<br>tivity<br>(D = 1.8) | Point Gamma             |                   |                   | at 1/10.<br>over | Cross-           |                   |               | Visual           |            |  |  |
|--------------------|-------------------------------|-------------------------|-------------------|-------------------|------------------|------------------|-------------------|---------------|------------------|------------|--|--|
|                    |                               | Average                 |                   | logE<br>(D = 1.8) |                  | CTF              |                   | Evaluation    |                  |            |  |  |
|                    |                               | Gradient<br>D = 1.6-2.0 | at<br>D = 1.6-2.0 |                   |                  | 1 line<br>per mm | 3 lines<br>per mm | Lung<br>Field | Medias-<br>tinum |            |  |  |
| 1                  | 316                           | 2.85                    | 2.7-3.0           | 0.15              | 12               | 0.79             | 0.42              | C             | Cz               | comparison |  |  |
| 2                  | 455                           | 2.75                    | 2.6-2.9           | 0.18              | 12               | 0.78             | 0.41              | Cz            | C                | comparison |  |  |
| 3                  | 223                           | 3.0                     | 2.9-3.2           | 0.12              | 12               | 0.79             | 0.42              | B             | Cz               | comparison |  |  |
| 4                  | 100                           | 3.85                    | 3.7-4.0           | 0.08              | 13               | 0.78             | 0.41              | Aa            | D                | comparison |  |  |
| 5                  | 177                           | 3.6                     | 3.5-3.8           | 0.10              | 13               | 0.77             | 0.40              | A             | D                | comparison |  |  |
| 6                  | 70                            | 3.9                     | 3.6-4.1           | 0.07              | 13               | 0.78             | 0.41              | Aa            | D                | comparison |  |  |
| 7                  | 102                           | 3.6                     | 3.5-3.7           | 0.31              | 13               | 0.78             | 0.41              | Aa            | B                | invention  |  |  |
| 8                  | 104                           | 3.4                     | 3.35-3.45         | 0.35              | 13               | 0.78             | 0.41              | A             | A                | invention  |  |  |
| 9                  | 106                           | 3.2                     | 3.0-3.3           | 0.40              | 13               | 0.78             | 0.41              | Az            | A                | invention  |  |  |
| 0                  | 110                           | 2.75                    | 2.5-2.9           | 0.50              | 13               | 0.77             | 0.40              | B             | Aa               | comparison |  |  |
| 11                 | 115                           | 2.4                     | 2.2-2.5           | 0.55              | 13               | 0.77             | 0.40              | C             | Aa               | comparison |  |  |
| 12                 | 130                           | 3.4                     | 3.35-3.45         | 0.35              | 25               | 0.70             | 0.32              | C             | B                | comparison |  |  |
| 13                 | 100                           | 3.4                     | 3.35-3.45         | 0.35              | 7                | 0.80             | 0.44              | Aa            | A                | invention  |  |  |
| 14                 | 190                           | 3.0                     | 2.9-3.1           | 0.35              | 12               | 0.78             | 0.41              | B             | Az               | invention  |  |  |
| 15                 | 195                           | 2.9                     | 2.8-3.0           | 0.40              | 12               | 0.78             | 0.41              | B             | B                | invention  |  |  |
| 16                 | 205                           | 2.6                     | 2.4-2.7           | 0.55              | 12               | 0.78             | 0.41              | C             | Ba               | comparison |  |  |
| 17                 | 240                           | 3.0                     | 2.9-3.1           | 0.38              | 24               | 0.69             | 0.31              | Cz            | B                | comparison |  |  |
| 18                 | 180                           | 3.0                     | 2.9-3.1           | 0.35              | 6                | 0.79             | 0.44              | Ba            | Ba               | invention  |  |  |
| 19                 | 72                            | 3.55                    | 3.2-3.7           | 0.40              | 13               | 0.78             | 0.42              | Aa            | Aa               | invention  |  |  |
| 20                 | 90                            | 3.55                    | 3.2-3.7           | 0.40              | 26               | 0.70             | 0.33              | Ca            | A                | Comparison |  |  |
| 21                 | 68                            | 3.55                    | 3.2-3.7           | 0.40              | 7                | 0.81             | 0.44              | Aa            | Aa               | invention  |  |  |

## [9] Image Evaluation using Thorax Phantom

Photographs were taken under a condition such that at the back of a thorax phantom, the products of Kyoto Kagaku K.K., a scattered rays cut filter having a grid ratio of 8:1 and an image-forming system constituted of a photosensitive material and intensifying screens were placed in that order, and the image-forming system was exposed via the thorax phantom by means of an X-ray source placed at a distance

60 The following were made clear by the data set forth in Table 5:

(1) The photosensitive materials according to the present invention, Sample Nos. 7, 8, 9, 13, 14, 15, 18, 19 and 21, have proved to have better depiction balance between the lung field and mediastinal area, compared with the photosensitive materials for comparison, Sample Nos. 1 to 6 and Sample Nos. 10, 11 and 16. More specifically, the samples

(Nos. 1 to 6) having a low point gamma value in the low exposure area (the area to which one-tenth the exposure amount required for providing the density of 1.8 was given) were inferior in depiction of mediastinal area. Conversely, the samples (Nos. 10, 11 and 16) having a satisfactory point gamma value in the low exposure area, but having low point gamma values in the medium density area ( $D=1.6-2.0$ ), were inferior in depiction of the lung field. Moreover, the CTF of the present samples had proved to be on a satisfactory level.

(2) The samples having a high crossover rate were low in CTF and inferior in depiction of the lung field even when

images which enabled satisfactory diagnosis. That is, the present samples have proved to be wide in exposure latitude.

(2) The Sample No. 4 was inferior in depiction of mediastinum and provided a photograph flat in the lung field under overexposure (+15%) since it had hard photographic characteristics.

(3) The Sample No. 10 was somewhat unsatisfactory in depiction of lung field, because in the density region  $D=1.6-2.0$  it had the point gamma values out of the scope of the present invention though it had the average gradient of 2.75. This tendency was particularly pronounced in case of underexposure (-15%).

TABLE 6

| Sam-<br>ple<br>No. | Exposure<br>Condition | Density at                   |               |                  | Vidual Evalution | Average | Point Gamma               |                     |                               | note |
|--------------------|-----------------------|------------------------------|---------------|------------------|------------------|---------|---------------------------|---------------------|-------------------------------|------|
|                    |                       | Fixed Point<br>in Lung Filed | Lung<br>Filed | Medias-<br>tinum |                  |         | Gradient<br>$D = 1.6-2.0$ | at<br>$D = 1.6-2.0$ | at 1/10.<br>$\log E(D = 1.8)$ |      |
| 4                  | -15%                  | 1.55                         | A             | D                |                  | 3.85    | 3.7-4.0                   | 0.08                | comparison                    |      |
|                    | ±0                    | 1.80                         | Aa            | D                |                  |         |                           |                     |                               |      |
|                    | +15%                  | 2.10                         | Bz            | Da               |                  |         |                           |                     |                               |      |
| 7                  | -15%                  | 1.58                         | A             | Bz               |                  | 3.6     | 3.5-3.7                   | 0.31                | invention                     |      |
|                    | ±0                    | 1.80                         | Aa            | B                |                  |         |                           |                     |                               |      |
|                    | +15%                  | 2.00                         | Az            | Ba               |                  |         |                           |                     |                               |      |
| 8                  | -15%                  | 1.60                         | A             | A                |                  | 3.4     | 3.35-3.45                 | 0.35                | invention                     |      |
|                    | ±0                    | 1.80                         | A             | A                |                  |         |                           |                     |                               |      |
|                    | +15%                  | 2.00                         | A             | Aa               |                  |         |                           |                     |                               |      |
| 9                  | -15%                  | 1.63                         | Az            | A                |                  | 3.2     | 3.0-3.3                   | 0.40                | invention                     |      |
|                    | ±0                    | 1.80                         | Az            | A                |                  |         |                           |                     |                               |      |
|                    | +15%                  | 1.95                         | Az            | Aa               |                  |         |                           |                     |                               |      |
| 10                 | -15%                  | 1.65                         | Ca            | Aa               |                  | 2.75    | 2.5-2.9                   | 0.50                | comparison                    |      |
|                    | ±0                    | 1.80                         | B             | Aa               |                  |         |                           |                     |                               |      |
|                    | +15%                  | 1.93                         | B             | Aa               |                  |         |                           |                     |                               |      |
| 11                 | -15%                  | 1.70                         | Cz            | Aa               |                  | 2.4     | 2.2-2.5                   | 0.55                | comparison                    |      |
|                    | ±0                    | 1.80                         | C             | Aa               |                  |         |                           |                     |                               |      |
|                    | +15%                  | 1.93                         | C             | Aa               |                  |         |                           |                     |                               |      |

they had the characteristic curve defined by the present invention (Sample Nos. 12, 17 and 20).

(3) In order to obtain the photosensitive materials according to the present invention, it has proved to be desirable that the support be provided with a dye layer for cutting crossover and the sensitivity ratio between the two emulsions used be approximately 3:1.

## EXAMPLE 2

In the same manner as in Example 1, images of thorax phantom were formed using the photosensitive materials chosen from those prepared in Example 1, that is, Sample No. 4, Sample No. 7 and Sample Nos. 8 to 11, respectively. In addition to the images formed under the exposure condition capable of providing the image density of 1.8 at one point chosen in the lung field (as adopted in Example 1), photographs of the same phantom were taken in the same manner as described above, except that the exposure condition was changed so as to increase or decrease the exposure amount by 15%.

The densities at the fixed point in the lung field were measured, and how the lung field and mediastinal area were depicted was evaluated by visual observation. The results obtained are shown in Table 6.

The data set forth in Table 6 have revealed the following.

(1) In the thorax image formation under the exposure conditions changed from the proper condition (lung field density: 1.8) so as to increase or decrease the exposure amount by 15%, the present samples (Nos. 7 to 9) provided

## EXAMPLE 3

## [1] Preparation of Intensifying Screen

In order to form a phosphor sheet, 200 g of a phosphor ( $Gd_2O_3:Tb$ ), 20 g of Binder A (polyurethane, Desmolack TPKL-5-2625 [solid portion: 40%], trade name, products of Sumitomo Bayer Urethane Co., Ltd.) and 2 g of Binder B (nitrocellulose having a nitrification degree of 11.5%) were added to methyl ethyl ketone as a solvent, and dispersed with a propeller mixer to prepare a coating composition (viscosity: 30 PS at 25°C, binder/phosphor ratio: 1/20). This coating composition was applied to a 180  $\mu\text{m}$ -thick polyethylene terephthalate film coated with a silicone type surface lubricant (temporary support) at a coverage such that the thickness of the coating might be 160  $\mu\text{m}$  after the compressive stressing treatment described hereinafter, dried and then peeled apart from the temporary support. Thus, a phosphor sheet was obtained.

Separately, a dispersion as a coating composition for forming a subbing layer was prepared by adding 90 g of a soft acrylic resin and 50 g of nitrocellulose to methyl ethyl ketone and mixing them. The dispersion obtained had a viscosity of 3-6 PS (at 25°C).

The coating composition for a subbing layer was uniformly spread over a 250  $\mu\text{m}$ -thick titanium dioxide-mixed polyethylene terephthalate film (support) placed horizontally on a glass plate, and then dried as the temperature of the glass plate was gradually raised from 25°C up to 100°C to form the subbing layer (thickness: 15  $\mu\text{m}$ ) on the support. On this subbing layer, the phosphor sheet prepared previ-

ously was superposed, and compressively stressed at 80° C. under the applied pressure of 400 Kg/cm<sup>2</sup> using a calender roll.

Further, a coating composition for forming a protective film was prepared by adding 70 g of a fluoro resin (fluorophlein-vinyl ether copolymer, Lumiflon LF 100, trade name, products of Asahi Glass Company, Ltd.), 25 g of a cross-linking agent (isocyanate, Desmodur Z 4370, trade name, products of Sumitomo Bayer Urethane Co., Ltd.), 5 g of bisphenol A type epoxy resin and 5 g of an alcohol-modified silicone oligomer (a silicone oligomer having a dimethylpolysiloxane skeleton and hydroxyl groups (carbinol groups) at the both ends, X-22-2809, trade name, products of Shin-etsu Chemical Industry Co., Ltd.) to a toluene-isopropyl alcohol (1:1 by volume) mixture as a solvent.

The thus prepared composition was coated on the surface of the phosphor sheet, which had previously undergone the compressive stressing treatment on the support, by means of a doctor blade, and then dried and thermally cured by 30 minute' heating at 120° C. Thus, a transparent protective film having a thickness of 3 μm was formed.

In the above-described manner, a Radiation Intensifying Screen A constituted of a support, a subbing layer, a phosphor layer and a transparent protective film was obtained.

#### Evaluation of Characteristics of Radiation Intensifying Screen

##### 1) Measurement of X-ray Absorption

X rays generated from a tungsten target tube operated by 80 KVp three-phase electric power supply were transmitted by a 3 mm-thick aluminum plate, and reached a radiation intensifying screen sample placed at a distance of 200 cm from the tungsten anode of the target tube. The amount of X rays transmitted by the intensifying screen sample was measured with an electric dissociation type dosimeter placed behind the phosphor layer of the intensifying screen at a distance of 50 cm. As for the standard, there was adopted the amount of X rays measured at the above-described position without being transmitted by any intensifying screen.

The data on the amount of X rays absorbed by each intensifying screen sample are shown in Table 7.

##### 2) Determination of Contrast Transfer Function (CTF)

A one-side photosensitive material MRE, products of Eastman Kodak Co., Ltd., was disposed in contact with each intensifying screen as subject of evaluation, and therein was formed the image of a rectangular chart for MTF measurement (made of molybdenum, having a thickness of 80 μm and spacial frequencies from 0 line/mm to 10 lines/mm). The rectangular chart was placed at a distance of 2 m from the X-ray tube. The X-ray source was arranged in front of the photosensitive material, and the intensifying screen sample was placed at the back of the photosensitive material. Herein, there were adopted the same X-ray source, photographic processing condition and CTF determination condition as used in Example 1.

In photographing, the exposure amount was controlled by changing the exposure time of X-rays so that the high density area of the resulting photograph might become 1.8. The results obtained are also shown in Table 7.

##### 3) Determination of Sensitivity

Each intensifying screen sample was combined with a green-sensitive one-side photosensitive material MRE, products of Eastman Kodak Co., Ltd., and exposed stepwise

by means of the same X-ray source as used in the determination of CTF. Therein, the amount of X rays was changed by a width of  $\log E=0.15$  at a step in accordance with a distance method. After the exposure, the photosensitive material underwent the same photographic processing operation as used in determining CTF values.

The density measurement of the thus processed photosensitive material was carried out using visible light, thereby obtaining a characteristic curve. The sensitivity was expressed in terms of the reciprocal of the exposure amount of X rays capable of providing the density of 1.8. The thus determined sensitivities of the intensifying screens are shown as relative values in Table 7, with the screen HR-4 for back-side arrangement being taken as 100.

TABLE 7

| Intensifying Screen   | Absorption of X rays | Sensitivity | CTF 1 line/mm | CTF 3 lines/mm |
|-----------------------|----------------------|-------------|---------------|----------------|
| HR-3 (front)          | 18.2%                | 48          | 0.890         | 0.660          |
| HR-3 (back)           | 18.2%                | 48          | 0.889         | 0.660          |
| HR-4 (front)          | 22.3%                | 89          | 0.850         | 0.510          |
| HR-4 (back)           | 23.1%                | 100         | 0.850         | 0.506          |
| HR-8 (front)          | 31.3%                | 155         | 0.775         | 0.340          |
| HR-8 (back)           | 32.2%                | 170         | 0.763         | 0.336          |
| Intensifying Screen A | 32.8%                | 200         | 0.869         | 0.494          |

As can be seen from Table 7, the Intensifying Screen A satisfies the requirements for achieving the satisfactory balance between the image quality and the sensitivity. These requirements are stated hereinbefore in connection with preferred embodiments of the present invention.

##### [2] Photosensitive Materials and Determination of Absolute Sensitivities Thereof

The absolute sensitivities of the samples prepared in Example 1 and those of commercial photosensitive materials Super HRS and Super HRC, trade names, products of Fuji Photo Film Co., Ltd., were examined respectively.

In examining the sensitivity, each photosensitive material was exposed by means of a tungsten light source having a color temperature of 2856° K. via a transmission filter having the transmission peak at 545 nm and the peak half-width of 20 nm (thereby the rays having their wavelength center at 545 nm, corresponding to the main emission wavelength of the radiation intensifying screen used hereinafter, were selectively taken out). Additionally, the exposure was carried out via a neutral step wedge, and the photosensitive material was irradiated with the selected rays for  $\frac{1}{20}$  second.

The exposed material was developed at 35° C. for 25 seconds (total processing time: 90 seconds) using Developer (I) in an automatic developing machine (FPM-5000, made by Fuji Photo Film Co., Ltd.). After the light-sensitive layer on the side opposite to the exposure side was peeled apart, density measurement was carried out to determine the characteristic curve. From the characteristic curve, the exposure amount necessary to provide the density of  $D_{min}$  (minimum density) plus 0.5 was calculated, and set forth in Table 8 as the sensitivity expressed in lux·sec. In calculating the exposure amount, the illuminance of the light emitted by the tungsten light source and transmitted by the filter was measured with an illuminometer, Model PI-3F (corrected).

TABLE 8

| Photosensitive Material                           | Sensitivity on one side<br>(D <sub>min</sub> + 0.5) |
|---------------------------------------------------|-----------------------------------------------------|
| Super HRS (product of Fuji Photo Film, Co., Ltd.) | 0.0076 lux.sec                                      |
| Super HRC (product of Fuji Photo Film Co., Ltd.)  | 0.0063 lux.sec                                      |
| Sensitive Material Sample No. 8                   | 0.0158 lux.sec                                      |
| Sensitive Material Sample No. 14                  | 0.0070 lux.sec                                      |
| Sensitive Material Sample No. 19                  | 0.0240 lux.sec                                      |
| Sensitive Material Sample No. 12                  | 0.0150 lux.sec                                      |
| Sensitive Material Sample No. 13                  | 0.0160 lux.sec                                      |

As can be seen from Table 8, the photosensitive materials 8, 19 and 13 had their respective sensitivities in the range specified in order to achieve the satisfactory balance between the image quality and the photographic speed. The sensitivity range requirement is stated hereinbefore in connection with preferred embodiments of the present invention. (Although the photosensitive material No. 12 met the sensitivity range requirement, it had too high crossover rate.)

[3] Sensitometry and Determination of Crossover Rate (%) and CTF

The combinations of the photosensitive materials with the intensifying screens, set forth in Table 9, were each examined for characteristic curve, crossover rate (%) and CTF values using the same methods as in Example 1.

The results obtained are shown in Table 9.

[4] Measurement of Noise Power Spectrum (NPS<sub>0</sub>(v))

Each combination of the photosensitive material with the intensifying screens was exposed by means of the same X-ray source as used in measurement of MTF (80 KVp, equipped with 3 mm-thick aluminum equivalent material and the filter of 7 cm-wide water) placed at a distance of 2 m. Therein, the exposure amount was controlled so as to provide a density of 1.0 when the photosensitive material was developed. The samples prepared for measurement of NPS<sub>0</sub> were scanned with a microdensitometer. The aperture used therein was a slit 30 μm wide in the scanning direction and 500 μm wide in the direction perpendicular to the

intervals of 20 μm. The 8192 (points/line)×12 (lines) sampling was carried out, and the sampled points were partitioned every 256 points, followed by undergoing a FFT processing. The average number of FFT was 1320 times. As a result of the FFT processing, the noise power spectrum was determined.

[5] Calculation of NEQ

The calculation of NEQ was made according to the following equation:

$$NEQ(v) = (\log_{10} \times \gamma \times MTF(v))^2 / NPS_0(v).$$

The NEQ values are shown as relative values, with the HR-4/Super HRS combination being taken as 100 (standard). As for the results obtained, the values at the spacial frequencies 1 line/mm and 3 lines/mm are shown as the representatives in Table 9.

[6] Calculation of DQE

The calculation of DQE was made according to the following equation:

$$DQE(v) = NEQ(v) / Q$$

(Q=quantum number of incident X rays).

As for the NEQ(v), the relative values determined above were used. Since Q is inversely proportional to the photographic speed of the combination of the photosensitive material with the intensifying screens, the foregoing equation can be converted to the following equation:

$$Relative DQE(v) = relative NEQ \times Relative Speed.$$

The relative DQE(v) values were calculated using the above equation, and they were shown as relative values with the HR-4/Super HRS combination being taken as 100 (standard). As for the results obtained, the values at the spacial frequencies 1 line/mm and 3 lines/mm are shown as the representatives.

[7] Evaluation of Image Quality using Thorax Phantom

Easiness in viewing the shadow of blood vessels in the lung field and the organs in the mediastinum was evaluated by the same method as in Example 1. The evaluation results are shown using the same marks as in Example 1.

TABLE 9

| Com-  | Inten- | Photo-    | ***  | Point Gamma |           | Cross- | CTF   |        | ***NEQ |        | ***DQE |        | Visual      |
|-------|--------|-----------|------|-------------|-----------|--------|-------|--------|--------|--------|--------|--------|-------------|
|       |        |           |      | Speed       | at        |        | over  | 1      | 3      | 1      | 3      | 1      | 3           |
| bina- | sify-  | sensi-    | (D = | D =         | 1/10.logE | Rate   | line/ | lines/ | line/  | lines/ | line/  | lines/ | lung        |
| tion  | ing    | tive      | 1.8) | 1.6-2.0     | (D = 1.8) | (%)    | mm    | mm     | mm     | mm     | mm     | mm     | filed       |
| No.   | Screen | Material  |      |             |           |        |       |        |        |        |        |        | mediastinum |
| 1     | HR-3   | Super HRS | 55   | 2.7-3.2     | 0.15      | 18     | 0.82  | 0.51   | 131    | 162    | 72     | 89     | Ba          |
| 2     | HR-4   | Super HRS | 100  | 2.8-3.2     | 0.15      | 18     | 0.72  | 0.37   | 100    | 100    | 100    | 100    | B           |
| 3     | HR-8   | Super HRS | 180  | 2.8-3.2     | 0.15      | 18     | 0.65  | 0.23   | 82     | 52     | 148    | 93     | C           |
| 4     | HR-4   | Super HRC | 120  | 2.4-2.6     | 0.43      | 22     | 0.69  | 0.34   | 80     | 75     | 96     | 90     | C           |
| **5   | A      | *8        | 110  | 3.3-3.6     | 0.35      | 13     | 0.75  | 0.35   | 160    | 115    | 176    | 127    | A           |
| **6   | A      | *19       | 73   | 3.2-3.7     | 0.40      | 13     | 0.75  | 0.35   | 230    | 171    | 173    | 125    | Aa          |
| 7     | A      | 12        | 140  | 3.3-3.6     | 0.35      | 25     | 0.68  | 0.30   | 121    | 86     | 170    | 120    | Bz          |
| **8   | A      | *13       | 105  | 3.3-3.6     | 0.35      | 7      | 0.76  | 0.36   | 172    | 129    | 181    | 135    | Aa          |
| 9     | HR-8   | *8        | 100  | 3.3-3.6     | 0.35      | 13     | 0.69  | 0.25   | 155    | 95     | 155    | 95     | Ba          |
| 10    | HR-8   | *19       | 60   | 3.2-3.7     | 0.40      | 13     | 0.69  | 0.25   | 253    | 155    | 152    | 93     | A           |
| 11    | HR-4   | *14       | 105  | 2.9-3.1     | 0.35      | 12     | 0.78  | 0.41   | 100    | 105    | 105    | 110    | B           |
| 12    | A      | *14       | 210  | 2.9-3.1     | 0.35      | 12     | 0.75  | 0.35   | 86     | 62     | 180    | 130    | Bz          |

In Table 9, the mark "\*" means that the photosensitive materials of the present invention were used, the mark "\*\*\*" means that the combinations are much preferable ones, and the mark "\*\*\*\*" means that the data are relative values with the HR-4/Super HRS combination being taken as 100.

scanning direction. The density was measured at sampling

The following has proved from the data set forth in Table

9:

(1) When the thorax images were formed using the present photosensitive materials 8, 13, 14 and 19, the depiction balance between the lung field and the mediastinum were very good, compared with Combination Nos. 1 to 4.

(2) Of the combinations according to the present invention, the combinations of the screen A produced for trial with the photosensitive materials having the specific sensitivity (Combination Nos. 5, 6 and 8) had improved DQE sensitivity on a standard level (73-100) and higher NEQ values than Combination No. 11, and were excellent in visual evaluation of the thorax image.

(3) Combination No. 7 using the photosensitive material 12 which had a high crossover rate although its characteristic curve was in the scope of the present invention was insufficient in CTF, and inferior particularly in depiction of the lung field.

(4) Combination No. 12 had high speed (210) because the intensifying screen therein had high sensitivity although the present photosensitive material having sensitivity on a standard level was used in combination, and provided a passable image of thorax in proportion for its high speed.

#### EXAMPLE 4

Each of the samples prepared in Example 1 was sandwiched between two sheets of HR-4 and exposed in the same manner as in Example 1, and processed using each of the following three kinds of processing systems, thereby evaluating photographic characteristics. For the evaluation of photographic characteristics, the speed at the density of 1.8, the point gamma values in the density range of 1.6 to 2.0 and the point gamma value at the exposure amount reduced to 1/10 the exposure amount required for providing the density of 1.8 were chosen as the representatives. Further, the evaluation of color stain in the film was made as follows: The photosensitive material measuring 24 cm×30 cm in size was subjected to each of the following three kinds of photographic processing operations without undergoing any exposure operation, and the color stain thereby generated was evaluated by visual observation.

##### Processing System I

Automatic Developing Machine FPM-5000 (produced by Fuji Photo Film Co., Ltd.) was used.

| Processing Step                                       | Time    | Temperature |
|-------------------------------------------------------|---------|-------------|
| Development with Developer I (described hereinbefore) | 25 sec. | 35° C.      |
| Fixation with Fixer F (described hereinbefore)        | 20 sec. | 25° C.      |
| Washing                                               | 12 sec. | 25° C.      |
| Drying                                                | 26 sec. | 55° C.      |

(Total processing time: 90 sec.)

##### Processing System II

An automatic developing machine, Fuji X-ray Processor Cepros M, produced by Fuji Photo Film Co., Ltd., was used.

| Processing Step               | Time      | Temperature |
|-------------------------------|-----------|-------------|
| Development with Developer II | 13.7 sec  | 35° C.      |
| Fixation with Fixer           | 10.6 sec  | 25° C.      |
| Washing                       | 6.2 sec.  | 25° C.      |
| Drying                        | 14.1 sec. | 55° C.      |

(Total processing time: 45 sec.)

| Composition of Developer II                      |        |  |
|--------------------------------------------------|--------|--|
| Potassium hydroxide                              | 18.0 g |  |
| Potassium sulfite                                | 75.0 g |  |
| Sodium carbonate                                 | 3.0 g  |  |
| Boric acid                                       | 5.0 g  |  |
| Diethylene glycol                                | 10.0 g |  |
| Diethylenetriaminepentaacetic acid               | 2.0 g  |  |
| 1-(N,N-Diethylamino)-ethyl-5-mercaptopentazole   | 0.1 g  |  |
| Hydroquinone                                     | 27.0 g |  |
| 4-Hydroxymethyl-4-methyl-1-phenyl-3-pyrazolidone | 2.0 g  |  |
| Triethylene glycol                               | 45.0 g |  |
| 3,3'-dithiobis(hydroxy)succinic acid             | 0.2 g  |  |
| Glacial acetic acid                              | 5.0 g  |  |
| 5-nitroindazole                                  | 0.3 g  |  |
| 1-Phenyl-3-pyrazolidone                          | 2.0 g  |  |
| Glutaraldehyde (50%)                             | 10.0 g |  |
| Potassium bromide                                | 1.0 g  |  |
| Potassium metabisulfite                          | 10.0 g |  |
| Water to make                                    | 1 l    |  |
| pH adjusted to                                   | 10.5   |  |

| Composition of Fixer G                         |        |  |
|------------------------------------------------|--------|--|
| Ammonium thiosulfate (70 wt/vol %)             | 200 ml |  |
| Disodium ethylenediaminetetraacetate dihydrate | 0.03 g |  |
| Sodium sulfite                                 | 15.0 g |  |
| Boric acid                                     | 4.0 g  |  |
| 1-(N,N-Diethylamino)-ethyl-5-mercaptopentazole | 1.0 g  |  |
| Tartaric acid                                  | 3.0 g  |  |
| Sodium hydroxide                               | 15.0 g |  |
| Sulfuric acid (36 N)                           | 3.9 g  |  |
| Aluminum sulfate                               | 10.0 g |  |
| Water to make                                  | 1 l    |  |
| pH adjusted to                                 | 4.60   |  |

##### Processing System III

A remodeling Fuji X-Ray Processing Cepros M was used as automatic developing machine.

| Processing Step                | Time     | Temperature |
|--------------------------------|----------|-------------|
| Development with Developer III | 9.1 sec. | 35° C.      |
| Fixation with Fixer G          | 7.1 sec. | 25° C.      |
| Washing                        | 4.1 sec. | 25° C.      |
| Drying                         | 9.4 sec  | 55° C.      |

(Total processing time: 30 sec.)

Developer III was the same as Developer II, except that the amounts of sodium carbonate and 1-phenyl-3-pyrazolidone used were changed to 30 g and 3.5 g respectively.

In remodelling the developing machine, the driving shaft was reconstructed so that the total processing time might be reduced to 30 seconds.

TABLE 10

| Processing               | Photo-sensitive          | Point Gamma |          |           | Color          | Coverage               |    |
|--------------------------|--------------------------|-------------|----------|-----------|----------------|------------------------|----|
|                          |                          | System      | Material | Speed     | at D = 1.6-2.0 | at 1/10.logE (D = 1.8) |    |
| (90 seconds' processing) | I                        | 8           | 104      | 3.35-3.45 | 0.35           | A                      | 25 |
|                          |                          | 12          | 130      | 3.35-3.45 | 0.35           | A                      | 0  |
|                          |                          | 13          | 100      | 3.35-3.45 | 0.35           | A                      | 40 |
|                          | II                       | 8           | 102      | 3.25-3.5  | 0.30           | A                      | 25 |
|                          | (45 seconds' processing) | 12          | 128      | 3.25-3.5  | 0.30           | A                      | 0  |
|                          |                          | 13          | 98       | 3.25-3.5  | 0.30           | A                      | 40 |
| (90 seconds' processing) | III                      | 8           | 100      | 3.3-3.6   | 0.35           | A                      | 25 |
|                          |                          | 12          | 126      | 3.3-3.6   | 0.35           | A                      | 0  |
|                          |                          | 13          | 97       | 3.3-3.6   | 0.35           | Az                     | 40 |

\*A: no color stain.

Az: slight color stain, but no problem in practical use.

As can be seen from Table 10, almost the same photographic characteristics as obtained in 90 seconds' processing were achieved in not only 45 second' processing but also 30 second' processing. As for the color stain in the film, on the other hand, there was no problem from the practical point of view even when Sample Nos. 8 and 13, which contained a dye in the support, were used as photosensitive material and the rapid processing, namely 45 seconds' processing and 30 second' processing, was carried out.

What is claimed is:

1. A radiation image-formation system comprising a silver halide photographic material for X-ray photography which has at least one light-sensitive silver halide emulsion layer on each side of a transparent support and two radiation-intensifying screens respectively arranged on the front and the back sides of the photographic material; said photographic material having a crossover rate of at most 15% with respect to the light emitted from said intensifying screens; and when sandwiched between two intensifying screens having substantially the same sensitivity, subjected to stepwise exposure and then developed with Developer (I) having the following composition at a developer temperature of 35° C. for a development time of 25 seconds, said photographic material producing an image having a characteristic curve such that when drawn using crossed coordinates equal to each other in unit length, with diffusion density as ordinate (Y-axis) and common logarithm of exposure amount as abscissa (X-axis), the characteristic curve provides a point gamma value ranging from 2.7 to 4.2 at every point within the optical density (diffusion density) range of 1.6 to 2.0 and a point gamma value of at least 0.25 at the density point corresponding to  $1/10$  of the exposure amount (-1.0 on logarithmic scale) required for providing the optical density of 1.8:

20

-continued

| Composition of Developer (I) |        |
|------------------------------|--------|
| 5-Methylbenzotriazole        | 0.05 g |
| Glutaraldehyde               | 5 g    |
| Potassium bromide            | 4 g    |
| Water to make                | 1 l    |
| pH adjusted to               | 10.02; |

wherein the light-sensitive emulsion layer arranged at least on either the front or the back side of the support has sensitivity requiring an exposure amount ranging from 0.010 lux-sec to 0.035 lux-sec to provide the density of minimum density plus 0.5 for said layer when the photographic material is exposed to monochromatic light having the same wavelength as that of the main emission peak of the radiation intensifying screens and a half width of  $20\pm 5$  nm, and developed with Developer (I) under a condition that a developer temperature is regulated at 35° C. and a development time is set at 25 seconds, and examined for the image density after the light-sensitive layer disposed on the opposite side is removed;

wherein at least one of said intensifying screens has at least 25% of absorption with respect to X rays having an energy of 80 KVp and contrast transfer function (CTF) values of at least 0.79 at the spacial frequency of 1 line/mm and at least 0.36 at the spacial frequency of 3 lines/mm.

2. The radiation image-formation system of claim 1, wherein at least one dye layer having a thickness of 0.5  $\mu$ m or less which enables reduction of crossover is provided between the silver halide emulsion layer and the support.

3. The radiation image-formation system of claim 1, wherein at least two kinds of silver halide emulsions constitute the light-sensitive silver halide emulsion layers and the ratio between the sensitivity of the silver halide emulsion having the highest sensitivity and the sensitivity of at least one among other emulsions is in the range of 1:0.5 to 1:0.15.

4. The radiation image-formation system of claim 3, wherein at least one of the silver halide emulsions comprises silver halide grains having a monodisperse grain size distribution the variation coefficient of which is 20% or less.

5. The radiation image-formation system of claim 1, wherein the light-sensitive silver halide emulsion layer comprises at least one kind of tabular silver halide grain emulsions.

6. The radiation image-formation system of claim 1, wherein the content of silver in the light-sensitive silver halide emulsion layer is at most 2  $\text{g}/\text{m}^2$  per each side.

| Composition of Developer (I) |       |
|------------------------------|-------|
| Potassium hydroxide          | 21 g  |
| Potassium sulfite            | 63 g  |
| Boric acid                   | 10 g  |
| Hydroquinone                 | 25 g  |
| Triethylene glycol           | 20 g  |
| 5-Nitroindazole              | 0.2 g |
| Glacial acetic acid          | 10 g  |
| 1-Phenyl-3-pyrazolidone      | 1.2 g |

7. A radiation image-formation system as in claim 1, wherein the radiation-intensifying screens have a phosphor layer, and phosphor for forming the phosphor layer is represented by the following formula:



wherein M represents at least one metal selected from the group consisting of yttrium, lanthanum, gadolinium and lutetium; M' represents at least one rare earth element; X represents an intermediate chalcogen or a halogen; n is a numerical value ranging from 0.0002 to 0.2; w is 1 when X is a halogen, and w is 2 when X is a chalcogen.

8. A radiation image-formation system as in claim 7, wherein the phosphor is selected from the group consisting of terbium-activated rare earth metal oxysulfide phosphors, terbium-activated rare earth element oxyhalogenide phosphors and thulium-activated rare earth element oxyhalogenide phosphors.

9. A method of forming radiation images using a silver halide photographic material which has at least one light-sensitive halide emulsion layer on each side of a transparent support; said photographic material having a crossover rate of at most 15% with respect to the light emitted from said intensifying screens; and when sandwiched between two intensifying screens having substantially the same sensitivity, subjected to stepwise exposure and then developed with Developer (I) having the following composition at a developer temperature of 35° C. for a development time of 25 seconds, said photographic material producing an image having a characteristic curve such that when drawn using crossed coordinates equal to each other in unit length, with diffusion density as ordinate (Y-axis) and common logarithm of exposure amount as abscissa (X-axis), the characteristic curve provides a point gamma value ranging from 2.7 to 4.2 at every point within the optical density (diffusion density) range of 1.6 to 2.0 and a point gamma value of at least 0.25 at the density point corresponding to  $1/10$  of the exposure amount (-1.0 on logarithmic scale) required for providing the optical density of 1.8:

-continued

| Composition of Developer (I) |                                                                                                                                                   |                                                        |
|------------------------------|---------------------------------------------------------------------------------------------------------------------------------------------------|--------------------------------------------------------|
| 5                            | Glacial acetic acid<br>1-Phenyl-3-pyrazolidone<br>5-Methylbenzotriazole<br>Glutaraldehyde<br>Potassium bromide<br>Water to make<br>pH adjusted to | 10 g<br>1.2 g<br>0.05 g<br>5 g<br>4 g<br>1 l<br>10.02; |

wherein the light-sensitive emulsion layer arranged at least on either the front or the back side of the support has sensitivity requiring an exposure amount ranging from 0.010 lux-sec to 0.035 lux-sec to provide the density of minimum density plus 0.5 for said layer when the photographic material is exposed to monochromatic light having the same wavelength as that of the main emission peak of the radiation intensifying screens and a half width of  $20\pm 5$  nm, and developed with Developer (I) under a condition that a developer temperature is regulated at 35° C. and a development time is set at 25 seconds, and examined for the image density after the light-sensitive layer disposed on the opposite side is removed; and sandwiching said material between two sheets of radiation intensifying screens at least one of which has at least 25% of absorption with respect to X rays having an energy of 80 KVp and contrast transfer function (CTF) values of at least 0.79 at the spacial frequency of 1 line/mm and at least 0.36 at the spacial frequency of 3 lines/mm.

10. The method of forming radiation images of claim 9, wherein the radiation-intensifying screen is basically constituted of a support and a phosphor layer formed on one side thereof.

11. The method of forming radiation images of claim 10, wherein the phosphor for forming the phosphor layer is  $Gd_2O_3:S:Tb$ .

12. The method of forming radiation images of claim 10, wherein a transparent protective layer is further provided on the surface of the phosphor layer at the side opposite to the support.

13. The method of forming radiation images of claim 12, wherein the transparent protective layer has a thickness of 5  $\mu m$  or less.

14. The method of forming radiation images of claim 10, wherein the radiation-intensifying screen is formed by compressively stressing a phosphor sheet on the support without previous fixation.

\* \* \* \* \*

## Composition of Developer (I)

|                     |       |
|---------------------|-------|
| Potassium hydroxide | 21 g  |
| Potassium sulfite   | 63 g  |
| Boric acid          | 10 g  |
| Hydroquinone        | 25 g  |
| Triethylene glycol  | 20 g  |
| 5-Nitrolindazole    | 0.2 g |